



US012146204B2

(12) **United States Patent**  
**Hirashima et al.**

(10) **Patent No.:** **US 12,146,204 B2**  
(45) **Date of Patent:** **Nov. 19, 2024**

(54) **STEEL SHEET, MEMBER, AND METHODS FOR PRODUCING THE SAME**

(71) Applicant: **JFE Steel Corporation**, Tokyo (JP)

(72) Inventors: **Takuya Hirashima**, Tokyo (JP); **Shimpei Yoshioka**, Tokyo (JP); **Shinjiro Kaneko**, Tokyo (JP); **Soshi Yoshimoto**, Tokyo (JP); **Tomohiro Hashimukai**, Tokyo (JP)

(73) Assignee: **JFE Steel Corporation**, Tokyo (JP)

(\*) Notice: Subject to any disclaimer, the term of this patent is extended or adjusted under 35 U.S.C. 154(b) by 444 days.

(21) Appl. No.: **17/769,829**

(22) PCT Filed: **Oct. 23, 2020**

(86) PCT No.: **PCT/JP2020/039950**

§ 371 (c)(1),  
(2) Date: **Apr. 18, 2022**

(87) PCT Pub. No.: **WO2021/085335**

PCT Pub. Date: **May 6, 2021**

(65) **Prior Publication Data**

US 2022/0364198 A1 Nov. 17, 2022

(30) **Foreign Application Priority Data**

Oct. 31, 2019 (JP) ..... 2019-198934

(51) **Int. Cl.**  
**C21D 9/50** (2006.01)  
**C21D 6/00** (2006.01)

(Continued)

(52) **U.S. Cl.**  
CPC ..... **C21D 9/505** (2013.01); **C21D 6/002** (2013.01); **C21D 6/005** (2013.01); **C21D 6/008** (2013.01);

(Continued)

(58) **Field of Classification Search**

CPC ..... C21D 9/505; C21D 6/002; C21D 6/005; C21D 6/008; C21D 8/0205; C21D 8/0226;

(Continued)

(56)

**References Cited**

U.S. PATENT DOCUMENTS

2015/0086808 A1 3/2015 Kasuya et al.  
2015/0368742 A1 12/2015 Shibata et al.

(Continued)

FOREIGN PATENT DOCUMENTS

CN 103703157 A 4/2014  
CN 104204259 A 12/2014

(Continued)

OTHER PUBLICATIONS

Chinese Office Action with Search Report for Chinese Application No. 202080074121.4, dated Sep. 15, 2022, 12 pages.

(Continued)

*Primary Examiner* — Adil A. Siddiqui

(74) *Attorney, Agent, or Firm* — Buchanan Ingersoll & Rooney PC

(57) **ABSTRACT**

The steel sheet of the present invention has a steel microstructure containing, in area fraction, martensite: 20% to 100%, ferrite: 0% to 80%, and another metal phase: 5% or less, in which, on a surface of the steel sheet, a ratio of dislocation density in metal phases at a widthwise edge of the steel sheet to dislocation density in the metal phases at a widthwise center of the steel sheet is 100% to 140%, and, at a thicknesswise center of the steel sheet, a ratio of dislocation density in the metal phases at the widthwise edge of the steel sheet to dislocation density in the metal phases at the widthwise center of the steel sheet is 100% to 140%.

(Continued)



The maximum amount of warpage of the steel sheet when the steel sheet is sheared to a length of 1 m in a rolling direction is 15 mm or less.

**14 Claims, 2 Drawing Sheets**

C22C 38/12; C22C 38/14; C22C 38/16;  
C22C 38/18; C22C 38/60; C22C 38/34;  
C22C 38/38; C22C 38/20; C22C 38/22;  
C22C 38/24; C22C 38/32; C22C 38/26;  
C22C 38/28; C22C 38/58

See application file for complete search history.

| (51) Int. Cl.     |           |
|-------------------|-----------|
| <i>C21D 8/02</i>  | (2006.01) |
| <i>C21D 9/42</i>  | (2006.01) |
| <i>C22C 38/00</i> | (2006.01) |
| <i>C22C 38/02</i> | (2006.01) |
| <i>C22C 38/04</i> | (2006.01) |
| <i>C22C 38/06</i> | (2006.01) |
| <i>C22C 38/08</i> | (2006.01) |
| <i>C22C 38/12</i> | (2006.01) |
| <i>C22C 38/14</i> | (2006.01) |
| <i>C22C 38/16</i> | (2006.01) |
| <i>C22C 38/18</i> | (2006.01) |
| <i>C22C 38/60</i> | (2006.01) |

| (52) U.S. Cl. |                                                                                                                                                                                                                                                                                                                                                                                                                                                                                                                                                                                   |
|---------------|-----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| CPC .....     | <i>C21D 8/0205</i> (2013.01); <i>C21D 8/0226</i> (2013.01); <i>C21D 8/0236</i> (2013.01); <i>C21D 8/0263</i> (2013.01); <i>C21D 9/42</i> (2013.01); <i>C22C 38/001</i> (2013.01); <i>C22C 38/002</i> (2013.01); <i>C22C 38/008</i> (2013.01); <i>C22C 38/02</i> (2013.01); <i>C22C 38/04</i> (2013.01); <i>C22C 38/06</i> (2013.01); <i>C22C 38/08</i> (2013.01); <i>C22C 38/12</i> (2013.01); <i>C22C 38/14</i> (2013.01); <i>C22C 38/16</i> (2013.01); <i>C22C 38/18</i> (2013.01); <i>C22C 38/60</i> (2013.01); <i>C21D 2211/005</i> (2013.01); <i>C21D 2211/008</i> (2013.01) |
|               | <i>C21D 2211/005</i> (2013.01); <i>C21D 2211/008</i> (2013.01); <i>C21D 1/19</i> ; <i>C21D 1/60</i> ; <i>C21D 1/63</i> ; <i>C21D 8/005</i> ; <i>C21D 8/0252</i> ; <i>C21D 8/0273</i> ; <i>C21D 9/0068</i> ; <i>C21D 9/563</i> ; <i>C21D 9/564</i> ; <i>C21D 9/573</i> ; <i>C21D 9/46</i> ; <i>C21D 1/18</i> ; <i>C21D 8/0247</i> ; <i>C22C 38/001</i> ; <i>C22C 38/002</i> ; <i>C22C 38/008</i> ; <i>C22C 38/02</i> ; <i>C22C 38/04</i> ; <i>C22C 38/06</i> ; <i>C22C 38/08</i> ;                                                                                                 |

| (58) Field of Classification Search |                                                                                                                                                                                                                                                                                                                                                                                                                                                                                                                                                 |
|-------------------------------------|-------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| CPC .....                           | <i>C21D 8/0236</i> ; <i>C21D 8/0263</i> ; <i>C21D 9/42</i> ; <i>C21D 2211/005</i> ; <i>C21D 2211/008</i> ; <i>C21D 1/26</i> ; <i>C21D 1/19</i> ; <i>C21D 1/60</i> ; <i>C21D 1/63</i> ; <i>C21D 8/005</i> ; <i>C21D 8/0252</i> ; <i>C21D 8/0273</i> ; <i>C21D 9/0068</i> ; <i>C21D 9/563</i> ; <i>C21D 9/564</i> ; <i>C21D 9/573</i> ; <i>C21D 9/46</i> ; <i>C21D 1/18</i> ; <i>C21D 8/0247</i> ; <i>C22C 38/001</i> ; <i>C22C 38/002</i> ; <i>C22C 38/008</i> ; <i>C22C 38/02</i> ; <i>C22C 38/04</i> ; <i>C22C 38/06</i> ; <i>C22C 38/08</i> ; |

**(56)**

**References Cited**

**U.S. PATENT DOCUMENTS**

2017/0327926 A1 11/2017 Yoshimoto et al.  
2019/0010564 A1 1/2019 Yoshimoto et al.  
2021/0310092 A1 10/2021 Kohsaka et al.

**FOREIGN PATENT DOCUMENTS**

|    |               |         |
|----|---------------|---------|
| CN | 105074040 A   | 11/2015 |
| EP | 2738278 A1    | 6/2014  |
| EP | 3556881 A1    | 10/2019 |
| EP | 3770292 A1    | 1/2021  |
| EP | 3778949 A1    | 2/2021  |
| JP | 462733 B1     | 1/1971  |
| JP | 083678 A      | 1/1996  |
| JP | 08176884 A    | 7/1996  |
| JP | 2005015854 A  | 1/2005  |
| JP | 2005272988 A  | 10/2005 |
| JP | 2012229466 A  | 11/2012 |
| JP | 5644095 B2    | 12/2014 |
| JP | 2016183414 A  | 10/2016 |
| JP | 6094722 B2    | 3/2017  |
| JP | 2017119912 A  | 7/2017  |
| JP | 2018135552 A  | 8/2018  |
| JP | 2020019992 A  | 2/2020  |
| KR | 20150142791 A | 12/2015 |
| WO | 2019181950 A1 | 9/2019  |
| WO | 2019186989 A1 | 10/2019 |
| WO | 2020026838 A1 | 2/2020  |

**OTHER PUBLICATIONS**

Extended European Search Report for European Application No. 20 881 945.8, dated Oct. 10, 2022, 10 pages.

Korean Written Decision on Registration issued Jun. 26, 2024, for Korean Application No. 10-2022-7013106 with an English translation. (5 pages).

International Search Report and Written Opinion for International Application No. PCT/JP2020/039950, dated Dec. 28, 2020, 6 pages.

FIG. 1



FIG. 2



FIG. 3



FIG. 4



## STEEL SHEET, MEMBER, AND METHODS FOR PRODUCING THE SAME

### CROSS REFERENCE TO RELATED APPLICATIONS

This is the U.S. National Phase application PCT/JP2020/039950, filed Oct. 23, 2020, which claims priority to Japanese Patent Application No. 2019-198934 filed Oct. 31, 2019, the disclosures of these applications being incorporated herein by reference in their entireties for all purposes.

### FIELD OF THE INVENTION

The present invention relates to a steel sheet used preferably for automotive parts etc., to a member, and to methods for producing the same. More particularly, the invention relates to a steel sheet having high strength, excellent shape uniformity, and excellent shape fixability, to a member, and to methods for producing the same.

### BACKGROUND OF THE INVENTION

In recent years, from the viewpoint of global environmental conservation, the automobile industry as a whole is striving to improve the fuel efficiency of automobiles in order to reduce CO<sub>2</sub> emission. The most effective way to improve the fuel efficiency of automobiles is to reduce the weight of the automobiles by reducing the thicknesses of parts used. Therefore, in recent years, the amount of high strength steel sheets used as materials of automotive parts is increasing.

To obtain sufficient steel sheet strength, many steel sheets utilize martensite, which is a hard phase. However, when martensite is formed, the uniformity of the sheet shape deteriorates due to transformation strain. The deterioration in the uniformity of the sheet shape adversely affects dimensional accuracy during forming. Therefore, steel sheets are subjected to straightening such as levelling or skin pass rolling (temper rolling) in order to obtain desired dimensional accuracy. However, when strain is introduced by the levelling or skin pass rolling, shape fixability deteriorates, and dimensional accuracy during forming deteriorates. Therefore, the desired dimensional accuracy is not obtained. To prevent the deterioration in the shape fixability, it is necessary to prevent deterioration in the uniformity of the sheet shape during martensite transformation, and various techniques have been proposed.

For example, in Patent Literature 1, the shape fixability of a multi-phase steel sheet is improved by reducing its yield ratio and r-value. Specifically, in the multi-phase steel sheet having a microstructure containing ferrite or bainite as the phase with the highest volume fraction and martensite at a volume fraction of from 1% to 25%, crystal orientations are controlled, and at least one of the r-value in a rolling direction and the r-value in a direction perpendicular to the rolling direction is adjusted to 0.7 or less. Moreover, the yield ratio is adjusted to 70% or less. In this manner, an ultrahigh-strength steel sheet having good shape fixability is provided.

Patent Literature 2 provides a high-strength steel sheet having excellent shape fixability. The high strength steel sheet is composed of steel having a chemical composition satisfying, in mass %, C: 0.10 to 0.35%, Si: 0.5 to 3.0%, Mn: 1.5 to 4.0%, P: 0.100% or less, S: 0.02% or less, and Al: 0.010 to 0.5%. The high strength steel sheet contains polygonal ferrite at an area fraction of 0 to 5%, bainitic

ferrite at an area fraction of 5% or more, martensite at an area fraction of 5 to 20%, tempered martensite at an area fraction of 30 to 60%, and retained austenite at an area fraction of 5 to 20%, and the average grain size of prior austenite is 15  $\mu\text{m}$  or less.

Patent Literature 3 provides a technique for preventing deterioration in the shape of a steel sheet caused by martensite transformation during water quenching by restraining the steel sheet by rolls in water.

### PATENT LITERATURE

PTL 1: Japanese Unexamined Patent Application Publication No. 2005-272988

PTL 2: Japanese Unexamined Patent Application Publication No. 2012-229466

PTL 3: Japanese Patent No. 6094722

### SUMMARY OF THE INVENTION

Steel sheets used for automobile bodies are subjected to press working before use, and therefore shape uniformity and shape fixability are their essential properties. In recent years, the amount of high-strength steel sheets used as the materials of automotive parts is increasing. It is therefore necessary for the steel sheets to have high strength and excellent shape fixability.

With the technique disclosed in Patent Literature 1, excellent shape fixability is obtained by controlling the crystal orientations and the r-value. However, since the steel sheet is shaped in all directions during forming, the shape fixability may not be good in some shaping directions. Moreover, the volume fraction of martensite is small, and the strength level is low.

With the technique disclosed in Patent Literature 2, a steel sheet having excellent shape fixability and strength equivalent to that of aspects of the present invention is provided by reducing the yield ratio. However, with the technique provided, since the difference in dislocation density in metal phases in the width direction is not reduced, the shape fixability may be poor, and no description is given regarding the shapes.

With the technique disclosed in Patent Literature 3, the shape uniformity can be improved. However, with the technique provided, since the difference in dislocation density in metal phases in the width direction is not reduced, the shape fixability may be poor.

It is an object according to aspects of the present invention to provide a high-strength steel sheet having excellent shape uniformity and excellent shape fixability and also provide a member and methods for producing the same.

The term "high strength" means that the tensile strength TS in a tensile test performed at a strain rate of 10 mm/min-<sup>1</sup> according to JIS Z2241 (2011) is 750 MPa or higher.

The term "excellent shape uniformity" means that the maximum amount of warpage of the steel sheet sheared to a length of 1 m in the rolling direction is 15 mm or less.

The term "excellent shape fixability" means that, as for the yield ratio YR in a tensile test performed at a strain rate of 10 mm/minutes according to JIS Z2241(2011),  $\Delta\text{YR}$ , which is the difference between the YR at the widthwise center of the sheet and the YR at widthwise edges of the sheet, is from -3% to 3%.

To solve the foregoing problems, the present inventors have conducted extensive studies on the requirements for a steel sheet having a tensile strength of 750 MPa or more, excellent shape uniformity, and excellent shape fixability.

The inventors have found that, to obtain excellent shape fixability, it is necessary that, on the surface of the steel sheet, a ratio of a dislocation density in metal phases at a widthwise edge of the sheet to a dislocation density in the metal phases at a widthwise center of the sheet be from 100% to 140% and that, at the thicknesswise center of the sheet, a ratio of a dislocation density in the metal phases at the widthwise edge of the sheet to a dislocation density in the metal phases at the widthwise center of the sheet be from 100% to 140%. The inventors have also found that, when the volume fraction of martensite formed by rapid cooling is 20% or more, high strength is obtained. Since the martensite transformation during water cooling proceeds rapidly and nonuniformly, the transformation strain causes deterioration in the shape uniformity. The inventors have examined how to reduce the adverse effect due to the transformation strain and found that the shape uniformity of a sheet is improved by applying restraining force to the front and back sides of the sheet during martensite transformation. The inventors have also found that, by controlling the restraining conditions to reduce variations in dislocation density in metal phases in the width direction, a variation in yield ratio (YR) in the width direction is reduced, and good shape fixability is obtained.

As described above, the present inventors have conducted various studies to solve the foregoing problems and found that a high-strength steel sheet having excellent shape uniformity and excellent shape fixability can be obtained, and thus aspects of the present invention have been completed. Aspects of the present invention are summarized as follows.

[1] A steel sheet which has a steel microstructure containing:

in area fraction, martensite: from 20% to 100%, ferrite: from 0% to 80%, and another metal phase: 5% or less;

in which, on a surface of the steel sheet, a ratio of a dislocation density in metal phases at a widthwise edge of the steel sheet to a dislocation density in the metal phases at a widthwise center of the steel sheet is from 100% to 140%; and

in which, at a thicknesswise center of the steel sheet, a ratio of a dislocation density in the metal phases at the widthwise edge of the steel sheet to a dislocation density in the metal phases at the widthwise center of the steel sheet is from 100% to 140%,

wherein the maximum amount of warpage of the steel sheet when the steel sheet is sheared to a length of 1 m in a rolling direction is 15 mm or less.

[2] The steel sheet according to [1], which has a chemical composition containing, in mass %,

C: from 0.05% to 0.60%,

Si: from 0.01% to 2.0%,

Mn: from 0.1% to 3.2%,

P: 0.050% or less,

S: 0.0050% or less,

Al: from 0.005% to 0.10%, and

N: 0.010% or less, with the balance being Fe and incidental impurities.

[3] The steel sheet according to [2], in which the chemical composition further contains, in mass %, at least one selected from

Cr: 0.20% or less,

Mo: less than 0.15%, and

V: 0.05% or less.

[4] The steel sheet according to [2] or [3], in which the chemical composition further contains, in mass %, at least one selected from

Nb: 0.020% or less and

Ti: 0.020% or less.

[5] The steel sheet according to any one of [2] to [4], in which the chemical composition further contains, in mass %, at least one selected from

Cu: 0.20% or less and

Ni: 0.10% or less.

[6] The steel sheet according to any one of [2] to [5], in which the chemical composition further contains, in mass %, B: less than 0.0020%.

[7] The steel sheet according to any one of [2] to [6], in which the chemical composition further contains, in mass %, at least one selected from

Sb: 0.1% or less and

Sn: 0.1% or less.

[8] A member which is prepared by subjecting the steel sheet according to any one of [1] to [7] to at least one of forming and welding.

[9] A method for producing a steel sheet, which includes: a hot rolling step of heating a steel slab having the chemical composition according to any one of [2] to [7] and then hot-rolling the steel slab; and

an annealing step of holding a hot-rolled steel sheet obtained in the hot rolling step at an annealing temperature equal to or higher than  $A_{C1}$  temperature for 30 seconds or longer, then starting water quenching the hot-rolled steel sheet from a temperature equal to or higher than Ms temperature including water cooling to 100° C. or lower, and reheating the hot-rolled steel sheet to from 100° C. to 300° C.,

wherein, in a region in which a surface temperature of the steel sheet is equal to or lower than (Ms temperature +150° C.) during the water cooling in the water quenching in the annealing step, the steel sheet is restrained from front and back sides of the steel sheet using two rolls such that the following conditions (1) to (3) are satisfied, the two rolls being disposed with the steel sheet interposed therebetween:

(1) a depression amount of each of the two rolls is more than 0 mm and  $t$  mm or less, where  $t$  is a thickness of the steel sheet;

(2)  $Rn$  and  $rn$  are from 50 mm to 1000 mm, where  $Rn$  and  $rn$  are roll diameters of the respective two rolls; and

(3) an inter-roll distance between the two rolls is more than 0 mm and  $(Rn+rn+t)/16$  mm or less.

[10] A method for producing a steel sheet, which includes: a hot rolling step of heating a steel slab having the chemical composition according to any one of [2] to [7] and then hot-rolling the steel slab;

a cold rolling step of cold-rolling a hot-rolled steel sheet obtained in the hot rolling step; and

an annealing step of holding a cold-rolled steel sheet obtained in the cold rolling step at an annealing temperature equal to or higher than  $A_{C1}$  temperature for 30 seconds or longer, then starting water quenching the cold-rolled steel sheet from a temperature equal to or higher than Ms temperature including water cooling to 100° C. or lower, and reheating the cold-rolled steel sheet to from 100° C. to 300° C.,

wherein, in a region in which a surface temperature of the steel sheet is equal to or lower than (Ms temperature +150° C.) during the water cooling in the water quenching in the annealing step, the steel sheet is restrained from front and back sides of the steel sheet using two

rolls such that the following conditions (1) to (3) are satisfied, the two rolls being disposed with the steel sheet interposed therebetween:

- (1) a depression amount of each of the two rolls is more than 0 mm and  $t$  mm or less, where  $t$  is a thickness of the steel sheet;
- (2)  $R_n$  and  $r_n$  are from 50 mm to 1000 mm, where  $R_n$  and  $r_n$  are roll diameters of the respective two rolls; and
- (3) an inter-roll distance between the two rolls is more than 0 mm and  $(R_n+r_n+t)/16$  mm or less.

[11] A method for producing a member, which includes a step of subjecting the steel sheet produced by the steel sheet production method according to [9] or [10] to at least one of forming and welding.

Aspects of the present invention can provide a high-strength steel sheet having excellent shape uniformity and excellent shape fixability and can also provide a member and methods for producing the same. By applying the steel sheet according to aspects of the present invention to a structural member of an automobile, the steel sheet for the automobile can have both high strength and improved shape fixability. Specifically, aspects of the present invention can improve the performance of the automobile body.

#### BRIEF DESCRIPTION OF THE DRAWINGS

FIG. 1 is a schematic illustration of an example of a steel sheet restrained by two rolls from the front and back side of the steel sheet during water cooling in an annealing step.

FIG. 2 is an enlarged illustration showing a portion near the two rolls in FIG. 1.

FIG. 3 is a schematic illustration showing the depression amounts of the rolls.

FIG. 4 is a schematic illustration showing the inter-roll distance between the two rolls.

#### DETAILED DESCRIPTION OF EMBODIMENTS OF THE INVENTION

Embodiments of the present invention will next be described. However, the present invention is not limited to the following embodiments.

The steel sheet according to aspects of the present invention has a microstructure containing, in area fraction, martensite: from 20% to 100%, ferrite: from 0% to 80%, and other metal phases: 5% or less, in which, on a surface of the steel sheet, a ratio of a dislocation density in metal phases at a widthwise edge of the steel sheet to a dislocation density in the metal phases at a widthwise center of the steel sheet is from 100% to 140%, and in which, at a thicknesswise center of the steel sheet, a ratio of a dislocation density in the metal phases at the widthwise edge of the steel sheet to a dislocation density in the metal phases at the widthwise center of the steel sheet is from 100% to 140%. The maximum amount of warpage of the steel sheet when the steel sheet is sheared to a length of 1 m in a rolling direction is 15 mm or less. With the steel sheet satisfying the above conditions, the effects according to aspects of the invention can be obtained. Therefore, no particular limitation is imposed on the chemical composition of the steel sheet.

First, the steel microstructure of the steel sheet according to aspects of the present invention will be described. "%" for martensite, ferrite, and other metal phases in the following description of the steel microstructure means the "area fraction (%)" based on the total area of the steel microstructure of the steel sheet."

Martensite: from 20% to 100%

To obtain high strength, i.e.,  $TS \geq 750$  MPa, the area fraction of martensite based on the total area of the microstructure is 20% or more. If the area fraction of martensite is less than 20%, the amount of any of ferrite, retained austenite, pearlite, and bainite increases, and the strength is reduced. The total area fraction of martensite based on the total area of the microstructure may be 100%. The area fraction of martensite is the sum of the area fraction of fresh martensite that is as-quenched martensite and the area fraction of tempered martensite subjected to tempering. In accordance with aspects of the present invention, the martensite is a hard microstructure generated from austenite at a temperature equal to or lower than the martensite transformation start temperature (simply referred to also as  $Ms$  temperature), and the tempered martensite is a microstructure obtained by reheating and tempering the martensite.

Ferrite: from 0% to 80%

From the viewpoint of maintaining sufficient strength, the area fraction of ferrite based on the total area of the steel microstructure of the steel sheet is 80% or less. The area fraction may be 0%. In accordance with aspects of the present invention, the ferrite is a microstructure formed by transformation from austenite at a relatively high temperature and forming bcc crystal grains.

Other Metal Phases: 5% or Less

The steel microstructure of the steel sheet according to aspects of the present invention may contain incidental metal phases other than the martensite and ferrite. The allowable area fraction of the other metal phases is 5% or less. The other metal phases include retained austenite, pearlite, bainite, etc. The area fraction of the other metal phases may be 0%. The retained austenite is austenite that has not undergone martensite transformation and remains at room temperature. The pearlite is a microstructure composed of ferrite and acicular cementite. The bainite is a hard microstructure formed from austenite at a relatively low temperature (equal to or higher than the martensite transformation start temperature) and including acicular or plate-shaped ferrite and carbides dispersed therein.

Values measured by a method described in Examples are used as the values of the area fractions of the microstructures in the steel microstructure.

Specifically, first, a test sample is taken from a steel sheet so as to extend in the rolling direction of the steel sheet and a direction perpendicular to the rolling direction, and a cross section along the sheet thickness  $L$  and parallel to the rolling direction is polished to a mirror finish and etched with a nital solution to cause the microstructure to appear. The sample with the microstructure appearing therein is observed using a scanning electron microscope. A 16×15 lattice with a spacing of 4.8  $\mu\text{m}$  is placed on a region with actual lengths of 82  $\mu\text{m}$ ×57  $\mu\text{m}$  in an SEM image at a magnification of 1500 $\times$ , and the area fraction of martensite is examined using a point counting method in which the number of points on each phase is counted. The area fraction is the average of three area fractions determined in different SEM images at a magnifications of 1500 $\times$ . The measurement is performed at a depth of one-fourth the sheet thickness. Martensite is a white microstructure, and tempered martensite includes fine carbides precipitated therein. Ferrite is a black microstructure. Depending on the plane orientations of block grains and the degree of etching, internal carbides may be less likely to appear. In such a case, it is necessary to perform etching sufficiently to check the internal carbides.

The area fraction of the metal phases other than ferrite and martensite is computed by subtracting the total area fraction of ferrite and martensite from 100%.

Ratio of dislocation density in metal phases at widthwise edge of steel sheet to dislocation density in metal phases at widthwise center of steel sheet on surface of steel sheet: from 100% to 140%, and ratio of dislocation density in metal phases at widthwise edge of steel sheet to dislocation density in metal phases at widthwise center of steel sheet at widthwise center of steel sheet: from 100% to 140%

To obtain excellent shape fixability, it is necessary to reduce variations in the YR in the width direction of the steel sheet. To achieve this, it is necessary to reduce variations in the dislocation density in metal phases that correlates with the YR. As for the dislocation densities in the metal phases at positions along the thickness of the steel sheet, the dislocation density on the surface tends to be smallest, and the dislocation density at the center tends to be largest. It is therefore inferred that, when variations in the dislocation density in the metal phases in the width direction of the steel sheet are small both on the surface and at the center, the variations in the dislocation density in the metal phases in the width direction of the steel sheet are small at any position along the thickness of the steel sheet. To obtain excellent shape fixability, it is necessary that, on the surface of the steel sheet, the ratio of the dislocation density in the metal phases at the widthwise edges of the sheet to the dislocation density in the metal phases at the widthwise center of the sheet ((the dislocation density in the metal phases at the widthwise edges of the sheet/the dislocation density in the metal phases at the widthwise center of the sheet) be 140% or less. It is also necessary that, at the thicknesswise center of the steel sheet, the ratio of the dislocation density in the metal phases at the widthwise edges of the sheet to the dislocation density in the metal phases at the widthwise center of the sheet (the dislocation density in the metal phases at the widthwise edges of the sheet/the dislocation density in the metal phases at the widthwise center of the sheet) be 140% or less. The ratio on the surface of the steel sheet and the ratio at the thicknesswise center of the steel sheet are preferably 135% or less and more preferably 130% or less. However, after the steel sheet is held for annealing, heat easily escapes from the widthwise edges of the sheet during cooling to the quenching temperature, and microstructures other than martensite are likely to be formed at the widthwise edges. As a result, YR decreases and a variation in YR in the width direction of the steel sheet increases. To reduce the variation in YR, it is necessary that the restraining conditions for water quenching be set appropriately such that the dislocation density in the metal phases at the widthwise edges of the sheet is equal to or higher than the dislocation density in the metal phases at the widthwise central portion of the sheet. Therefore, it is necessary that, on the surface of the steel sheet, the ratio of the dislocation density in the metal phases at the widthwise edges of the sheet to the dislocation density in the metal phases at the widthwise center of the sheet be 100% or more and that, at the thicknesswise center of the steel sheet, the ratio of the dislocation density in the metal phases at the widthwise edges of the sheet to the dislocation density in the metal phases at the widthwise center of the sheet be 100% or more. The ratio on the surface of the steel sheet and the ratio at the thicknesswise center of the sheet are preferably 110% or more and more preferably 120% or more.

In accordance with aspects of the present invention, the surface of the steel sheet on which the dislocation density is

determined is meant to encompass both the front and back surfaces of the steel sheet (one surface and the other surface opposite thereto).

A value obtained by a method described in Examples is used as the ratio of the dislocation density in the metal phases at the widthwise edges of the sheet to the dislocation density in the metal phases at the widthwise center of the sheet.

Specifically, first, a sample with a width of 10 mm $\times$ 10 conveying direction length of 10 mm is taken from each of a widthwise central portion of a steel sheet and a widthwise edge portion of the steel sheet (an outermost edge portion of the steel sheet). The surface of each steel sheet sample is polished to remove scales, and the polished surface of the steel sheet is subjected to X-ray diffraction measurement. The amount of the steel sheet polished to remove scales is less than 1  $\mu\text{m}$ . The radiation source is Co. Since the analysis depth of Co is about 20  $\mu\text{m}$ , the dislocation density in the metal phases on the surface of the steel sheet is the dislocation density in the metal phases in the range of 0 to 20  $\mu\text{m}$  from the surface of the steel sheet. The dislocation density in the metal phases is determined using a method in which the dislocation density is converted from a strain determined using half widths  $\beta$  in the X-ray diffraction measurement. To extract the strain, the Williamson-Hall method described below is used. The half width is influenced by the size D of crystallites and the strain  $\epsilon$  and can be computed as the sum of these factors using the following formula.

$$\beta = \beta_1 + \beta_2 = (0.9\lambda/(D \times \cos \theta)) + 2\epsilon \tan \theta$$

By modifying this formula,  $\beta \cos \theta/\lambda = 0.9\lambda/D + 2\epsilon \sin \theta/\lambda$  is obtained.  $\beta \cos \theta/\lambda$  is plotted versus  $\sin \theta/\lambda$ , and the strain  $\epsilon$  is computed from the gradient of the straight line. The diffraction lines used for the computation are (110), (211), and (220). To convert the strain  $\epsilon$  to the dislocation density in the metal phases,  $\rho = 14.4\epsilon^2/b^2$  is used.  $\theta$  is a peak angle computed using the  $\theta-2\theta$  method for X-ray diffraction, and  $\lambda$  is the wavelength of the X-ray used for the X-ray diffraction. b is the Burgers vector of Fe( $\alpha$ ) and is 0.25 nm in accordance with aspects of the present invention. Then the ratio of the dislocation density in the metal phases on the surface of a widthwise edge of the steel sheet to the dislocation density in the metal phases on the surface of the widthwise center of the steel sheet on the surface of the steel sheet is determined.

A description will next be given of a method for computing the ratio of the dislocation density in the metal phases at a widthwise edge of a sheet to the dislocation density in the metal phases at the widthwise center of the sheet at the thicknesswise center of the sheet.

A sample with a width of 20 mm $\times$ 10 conveying direction length of 20 mm is taken from each of a widthwise central portion of a steel sheet and a widthwise edge portion of the sheet. The surface of each steel sheet sample is polished to remove scales. The amount of the steel sheet polished to remove scales is less than 1  $\mu\text{m}$ . Next, the surface of each sample is ground to the thicknesswise center of the sheet, and the resulting sample is subjected to X-ray diffraction measurement using the same method as that for the measurement on the surface of the steel sheet. Since the analysis depth of Co is about 20  $\mu\text{m}$ , the dislocation density in the metal phases at the thicknesswise center of the sheet is the dislocation density in the metal phases in the range of 0 to 20  $\mu\text{m}$  from the center of the steel sheet. Based on the results of the measurement, the ratio of the dislocation density in the metal phases on the surface of the widthwise edge of the

sheet to the dislocation density in the metal phases on the surface of the widthwise center of the sheet is determined.

In the thickness direction of the sheet, the dislocation density in the metal phases tends to be largest in the thicknesswise central portion of the sheet and tends to be smallest on the surface. Therefore, in accordance with aspects of the present invention, the dislocation density in the metal phases is measured on the surface and at the thicknesswise central portion of the sheet, and the measured dislocation densities are used to define the dislocation density ratios in the metal phases in the width direction at all thicknesswise positions of the sheet.

Next, the properties of the steel sheet according to aspects of the present invention will be described.

The steel sheet according to aspects of the present invention has excellent shape uniformity. Specifically, the maximum amount of warpage of the steel sheet when the steel sheet is sheared to a length of 1 m in the rolling direction (longitudinal direction) of the steel sheet is 15 mm or less. The maximum amount of warpage is preferably 10 mm or less and more preferably 8 mm or less. No limitation is imposed on the lower limit of the maximum amount of warpage, and the maximum amount of warpage is most preferably 0 mm.

The phrase "the maximum amount of warpage of the steel sheet when the steel sheet is sheared to a length of 1 m in the longitudinal direction" as used herein means as follows. The steel sheet is sheared to a length of 1 m in the steel sheet longitudinal direction (rolling direction) while the original width of the steel sheet is maintained. Then the sheared steel sheet is placed on a horizontal table. The distance from the horizontal table to the steel sheet at a position at which the gap between the horizontal table and a lower portion of the steel sheet is largest is used as the maximum amount of warpage. The above distance is the distance in a direction perpendicular to a horizontal surface of the horizontal table (the vertical direction). After the measurement of the amount of warpage with one surface of the steel sheet facing upward, the amount of warpage is measured with the other surface of the steel sheet facing upward, and the largest one of the measured warpage amounts is used as the maximum amount of warpage. The sheared steel sheet is placed on the horizontal table such that the horizontal table and the steel sheet are in contact with each other at as many corner portions of the steel sheet as possible (at two or more corner portions). The amount of warpage is determined by lowering a horizontal plate from a position higher than the steel sheet until the horizontal plate comes into contact with the steel sheet and subtracting the thickness of the steel sheet from the distance between the horizontal table and the horizontal plate at the contact position at which the horizontal plate is in contact with the steel sheet. When the steel sheet is sheared in the longitudinal direction, the clearance between the cutting edges of the shearing machine is set to 4% (the upper limit of the control range is 10%).

The strength of the steel sheet according to aspects of the present invention is high. Specifically, as described in Examples, the tensile strength determined by a tensile test performed at a strain rate of 10 mm/minutes according to JIS Z2241 (2011) is 750 MPa or more. The tensile strength is preferably 950 MPa or more, more preferably 1150 MPa or more, and still more preferably 1300 MPa or more. No particular limitation is imposed on the upper limit of the tensile strength. However, from the viewpoint of ease of achieving balance between the tensile strength and other properties, the tensile strength is preferably 2500 MPa or lower.

The steel sheet according to aspects of the present invention has excellent shape fixability. By reducing the variations in the yield strength (YR) in the width direction that correlates with the dislocation density in the metal phases, the shape fixability is improved. Specifically, as for the yield ratio YR measured using the tensile test performed at a strain rate of 10 mm/minutes according to JIS 22241 (2011) as described in the Examples, the variations in yield ratio ( $\Delta$ YR) determined by a method in which the difference between the YR at the widthwise center of the sheet and the YR at a widthwise edge of the sheet is determined is from -3% to 3%. The variations in yield ratio ( $\Delta$ YR) are preferably from -2% to 2% and more preferably from -1% to 1%.

From the viewpoint of obtaining the effects according to aspects of the invention effectively, the thickness of the steel sheet according to aspects of the present invention is preferably from 0.2 mm to 3.2 mm.

Next, a description will be given of a preferred chemical composition for obtaining the steel sheet according to aspects of the present invention. In the following description of the chemical composition, "%" used as the unit of the content of a component means "% by mass."

C: From 0.05% to 0.60%

C is an element that improves the hardenability. When C is contained, a prescribed area fraction of martensite can be easily obtained. Moreover, when C is contained, the strength of martensite is increased, and sufficient strength can be easily obtained. From the viewpoint of obtaining prescribed strength while excellent shape fixability is maintained, the content of C is preferably 0.05% or more. From the viewpoint of achieving  $TS \geq 950$  MPa, the content of C is more preferably 0.11% or more. From the viewpoint of achieving  $TS \geq 1150$  MPa, the content of C is preferably 0.125% or more. However, if the content of C exceeds 0.60%, not only the strength tends to be excessively high, but also transformation expansion due to martensite transformation is not easily prevented. In this case, the shape uniformity tends to deteriorate. Therefore, the content of C is preferably 0.60% or less. The content of C is more preferably 0.50% or less and still more preferably 0.40% or less.

Si: From 0.01% to 2.0%

Si is an element for strengthening through solid solution strengthening. To obtain this effect sufficiently, the content of Si is preferably 0.01% or more. The content of Si is more preferably 0.02% or more and still more preferably 0.03% or more. However, if the content of Si is excessively large, coarse MnS is likely to be formed in a widthwise central portion of the sheet. In this case, the dislocation density in the metal phases at the widthwise center of the sheet relative to the dislocation density at widthwise edges of the sheet decreases, and the shape fixability tends to deteriorate. Therefore, the content of Si is preferably 2.0% or less, more preferably 1.7% or less, and still more preferably 1.5% or less.

Mn: From 0.1% to 3.2%

Mn is contained in order to improve the hardenability of the steel and to obtain a prescribed area fraction of martensite. If the content of Mn is less than 0.1%, ferrite is formed in a surface layer portion of the steel sheet, and the strength tends to decrease. Therefore, the content of Mn is preferably 0.1% or more, more preferably 0.2% or more, and still more preferably 0.3% or more. Moreover, Mn is an element that particularly facilitates the formation and coarsening of MnS. If the content of Mn exceeds 3.2%, the amount of coarse inclusions increases, and coarse MnS is likely to be formed in the widthwise central portion of the sheet. In this case, the dislocation density in the metal phases at the widthwise

## 11

center of the sheet relative to the dislocation density at the widthwise edges of the sheet decreases, and the shape fixability tends to deteriorate. Therefore, the content of Mn is preferably 3.2% or less, more preferably 3.0% or less, and still more preferably 2.8% or less.

P: 0.050% or Less

P is an element that strengthens the steel. However, if the content of P is large, the occurrence of cracks is facilitated, and P tends to segregate at grain boundaries in the widthwise central portion of the sheet. In this case, the dislocation density in the metal phases at the widthwise center of the sheet relative to the dislocation density at the widthwise edges of the sheet decreases, and the shape fixability tends to deteriorate. Therefore, the content of P is preferably 0.050% or less, more preferably 0.030% or less, and still more preferably 0.010% or less. No particular limitation is imposed on the lower limit of the content of P. At present, the industrially achievable lower limit of P is about 0.003%.

S: 0.0050% or Less

S forms MnS, TiS, Ti(C, S), etc., and this is likely to cause the formation of coarse inclusions in the widthwise central portion of the sheet. In this case, the dislocation density in the metal phases at the widthwise center of the sheet relative to the dislocation density at the widthwise edges of the sheet decreases, and the shape fixability tends to deteriorate. To reduce the adverse effect of the inclusions, the content of S is preferably 0.0050% or less. The content of S is more preferably 0.0020% or less, still more preferably 0.0010% or less, and particularly preferably 0.0005% or less. No particular limitation is imposed on the lower limit of the content of S. At present, the industrially achievable lower limit of S is about 0.0002%.

Al: from 0.005% to 0.10%

Al is added to allow the steel to undergo deoxidization sufficiently to thereby reduce the amount of coarse inclusions in the steel. From the viewpoint of obtaining the effect of Al sufficiently, the content of Al is preferably 0.005% or more. The content of Al is more preferably 0.010% or more. If the content of Al exceeds 0.10%, carbides composed mainly of Fe such as cementite formed during coiling after hot rolling are unlikely to dissolve in an annealing step, and coarse inclusions and carbides tend to be formed. This easily causes not only a reduction in strength but also coarsening of the inclusions and carbides particularly in the widthwise central portion of the sheet. In this case, the dislocation density in the metal phases at the widthwise center of the sheet relative to the dislocation density at the widthwise edges of the sheet decreases, and the shape fixability tends to deteriorate. Therefore, the content of Al is preferably 0.10% or less, more preferably 0.08% or less, and still more preferably 0.06% or less.

N: 0.010% or Less

N is an element that forms nitrides such as TiN, (Nb, Ti) (C, N), and AlN and carbonitride-based coarse inclusions in the steel. The formation of these nitrides and inclusions is likely to cause the formation of coarse inclusions in the widthwise central portion of the sheet. In this case, the dislocation density in the metal phases at the widthwise center of the sheet relative to the dislocation density at the widthwise edges of the sheet decreases, and the shape fixability tends to deteriorate. To prevent deterioration in the shape fixability, the content of N is preferably 0.010% or less. The content of N is more preferably 0.007% or less and still more preferably 0.005% or less. No particular limitation is imposed on the lower limit of the content of N. At present, the industrially achievable lower limit of N is about 0.0006%.

## 12

The steel sheet according to aspects of the present invention has a chemical composition containing the above components with the balance other than the above components being Fe (iron) and incidental impurities. Preferably, the steel sheet according to aspects of the present invention has a chemical composition containing the above components with the balance being Fe and incidental impurities. The steel sheet according to aspects of the present invention may contain the following allowable components (optional elements) so long as the operation according to aspects of the invention is not impaired.

At least one selected from Cr: 0.20% or less, Mo: less than 0.15%, and V: 0.05% or less

Cr, Mo, and V can be contained for the purpose of obtaining the effect of improving the hardenability of the steel. However, if the content of any of these elements is excessively large, their carbides coarsen. In this case, the dislocation density in the metal phases at the widthwise center of the sheet relative to the dislocation density at the widthwise edges of the sheet decreases, and the shape fixability deteriorates. Therefore, the content of Cr is preferably 0.20% or less and more preferably 0.15% or less. The content of Mo is preferably less than 0.15% and more preferably 0.10% or less. The content of V is preferably 0.05% or less, more preferably 0.04% or less, and still more preferably 0.03% or less. No particular limitation is imposed on the lower limit of the content of Cr and the lower limit of the content of Mo. However, from the viewpoint of obtaining the effect of improving the hardenability more effectively, the content of Cr and the content of Mo are each preferably 0.01% or more. The content of Cr and the content of Mo are each more preferably 0.02% or more and still more preferably 0.03% or more. No particular limitation is imposed on the lower limit of the content of V. However, from the viewpoint of obtaining the effect of improving the hardenability more effectively, the content of V is preferably 0.001% or more. The content of V is more preferably 0.002% or more and still more preferably 0.003% or more.

At least one selected from Nb: 0.020% or less and Ti: 0.020% or less

Nb and Ti contribute to strengthening through refinement of prior- $\gamma$  grains. However, if large amounts of Nb and Ti are contained, the amount of Nb-based coarse precipitates such as NbN, Nb(C, N), and (Nb, Ti) (C, N) and Ti-based coarse precipitates such as TiN, Ti(C, N), Ti(C, S), and TiS that remain undissolved during slab heating in a hot rolling step increases. In this case, the dislocation density in the metal phases at the widthwise center of the sheet relative to the dislocation density at the widthwise edges of the sheet decreases, and the shape fixability deteriorates. Therefore, the content of Nb and the content of Ti are each preferably 0.020% or less, more preferably 0.015% or less, and still more preferably 0.010% or less. No particular limitation is imposed on the lower limit of the content of Nb and the lower limit of the content of Ti. However, from the viewpoint of obtaining the effect of increasing the strength more effectively, at least one of Nb and Ti is contained in an amount of 0.001% or more. The content of each of these elements is more preferably 0.002% or more and still more preferably 0.003% or more.

At least one selected from Cu: 0.20% or less and Ni: 0.10% or less

Cu and Ni have the effect of improving corrosion resistance in the use environment of automobiles and the effect of preventing intrusion of hydrogen into the steel sheet when their corrosion products cover the surface of the steel sheet. However, when the content of Cu and the content of Ni are

excessively large, surface defects occur, and coatability and chemical conversion processability necessary for steel sheets for automobiles deteriorate. Therefore, the content of Cu is preferably 0.20% or less, more preferably 0.15% or less, and still more preferably 0.10% or less. The content of Ni is preferably 0.10% or less, more preferably 0.08% or less, and still more preferably 0.06% or less. No particular limitation is imposed on the lower limit of the content of Cu and the lower limit of the content of Ni. However, from the viewpoint of obtaining the effect of improving corrosion resistance and the effect of preventing intrusion of hydrogen more effectively, at least one of Cu and Ni is contained in an amount of preferably 0.001% or more and more preferably 0.002% or more.

B: Less than 0.0020%

B is an element that improves the hardenability of the steel. When B is contained, even if the content of Mn is small, the effect of forming martensite with a prescribed area fraction is obtained. However, if the content of B is 0.0020% or more, the dissolution rate of cementite during annealing slows down, and carbides composed mainly of Fe such as undissolved cementite remain present. Therefore, coarse inclusions and carbides are formed. In this case, the dislocation density in the metal phases at the widthwise center of the sheet relative to the dislocation density at the widthwise edges of the sheet decreases, and the shape fixability tends to deteriorate. Therefore, the content of B is preferably less than 0.0020%, more preferably 0.0015% or less, and still more preferably 0.0010% or less. No particular limitation is imposed on the lower limit of the content of B. However, from the viewpoint of obtaining the effect of improving the hardenability of the steel more effectively, the content of B is preferably 0.0001% or more, more preferably 0.0002% or more, and still more preferably 0.0003% or more. From the viewpoint of fixing N, it is preferable to add Ti in an amount of 0.0005% or more in combination with B.

At least one selected from Sb: 0.1% or less and Sn: 0.1% or less

Sb and Sn inhibit oxidation and nitriding of the surface layer portion of the steel sheet to thereby prevent a reduction in the amounts of C and B due to oxidation and nitriding of the surface layer portion of the steel sheet. Since the reduction in the amounts of C and B is prevented, the formation of ferrite in the surface layer portion of the steel sheet is inhibited, and this contributes to an increase in the strength. However, if any of the content of Sb and the content of Sn exceeds 0.1%, Sb and Sn segregate at prior- $\gamma$  grain boundaries. In this case, the dislocation density in the metal phases at the widthwise center of the sheet relative to the dislocation density at the widthwise edges of the sheet decreases, and the shape fixability deteriorates. Therefore, each of the content of Sb and the content of Sn is preferably 0.1% or less. The content of Sb and the content of Sn are each more preferably 0.08% or less and still more preferably 0.06% or less. No particular limitation is imposed on the lower limit of the content of Sb and the lower limit of the content of Sn. However, from the viewpoint of obtaining the effect of increasing the strength more effectively, the content of each of Sb and Sn is preferably 0.002% or more. The content of Sb and the content of Sn are each more preferably 0.003% or more and still more preferably 0.004% or more.

The steel sheet according to aspects of the present invention may contain other elements including Ta, W, Ca, Mg, Zr, and REMs so long as the effects according to aspects of the invention are not impaired. The allowable content of each of these elements is 0.1% or less.

Next, a method for producing the steel sheet according to aspects of the present invention will be described.

The method for producing the steel sheet according to aspects of the present invention includes a hot rolling step, an optional cold rolling step, and an annealing step. One embodiment of the method for producing the steel sheet according to aspects of the present invention includes: the hot rolling step of heating a steel slab having the chemical composition described above and then hot-rolling the steel slab; the optional cold rolling step; and the annealing step of holding a hot-rolled steel sheet obtained in the hot rolling step or a cold-rolled steel sheet obtained in the cold rolling step at an annealing temperature equal to or higher than  $A_{C1}$  temperature for 30 seconds or longer, then starting water quenching from a temperature equal to or higher than  $M_s$  temperature to water-cool the resulting steel sheet to 100°C. or lower, and reheating the cooled steel sheet to from 100°C. to 300°C. In a region in which the surface temperature of the steel sheet is equal to or lower than ( $M_s$  temperature + 150°C.) during water cooling in the water quenching in the annealing step, the steel sheet is restrained from the front and back sides of the steel sheet using two rolls such that the following conditions (1) to (3) are satisfied, the two rolls being disposed with the steel sheet interposed therebetween:

- (1) the depression amount of each of the two rolls is more than 0 mm and  $t$  mm or less, where  $t$  is the thickness of the steel sheet;  
 (2)  $R_n$  and  $r_n$  are from 50 mm to 1000 mm, where  $R_n$  and  $r_n$  are the roll diameters of the respective two rolls; and  
 (3) the inter-roll distance between the two rolls is more than 0 mm and  $(R_n+r_n+t)/16$  mm or less.

Each of the steps will next be described. The temperatures described below when the steel slab, the steel sheet, etc. are heated or cooled are the surface temperatures of the steel slab, the steel sheet, etc., unless otherwise specified.

#### Hot Rolling Step

The hot rolling step is the step of heating the steel slab having the chemical composition described above and then hot-rolling the heated steel slab.

The steel slab having the chemical composition described above is subjected to hot rolling. No particular limitation is imposed on the heating temperature of the slab. When the heating temperature is 1200°C. or higher, dissolution of sulfides is facilitated, and the degree of segregation of Mn is reduced. In this case, the amount of the coarse inclusions described above and the amount of the carbides are reduced, and the shape fixability is improved. Therefore, the heating temperature of the slab is preferably 1200°C. or higher. The heating temperature of the slab is more preferably 1230°C. or higher and still more preferably 1250°C. or higher. No particular limitation is imposed on the upper limit of the heating temperature of the slab, but the heating temperature is preferably 1400°C. or lower. No particular limitation is imposed on the heating rate when the slab is heated, but the heating rate is preferably 5 to 15°C./minute. No particular limitation is imposed on the soaking time of the slab when the slab is heated, but the soaking time is preferably 30 to 100 minutes.

The temperature of finish rolling is preferably 840°C. or higher. If the finish rolling temperature is lower than 840°C., it takes time for the temperature to drop, and inclusions and coarse carbides are formed. In this case, not only the shape fixability may deteriorate, but also the interior quality of the steel sheet may deteriorate. Therefore, the finish rolling temperature is preferably 840°C. or higher. The finish rolling temperature is more preferably 860°C. or higher. No particular limitation is imposed on the upper limit

of the finish rolling temperature. However, to avoid difficulty in subsequent cooling to coiling temperature, the finish rolling temperature is preferably 950°C. or lower. The finish rolling temperature is more preferably 920°C. or lower.

Preferably, the hot-rolled steel sheet cooled to the coiling temperature is coiled at a temperature equal to or lower than 630°C. If the coiling temperature is higher than 630°C., the surface of the base iron may be decarburized. This may cause a difference in microstructure between the interior of the steel sheet and the surface of the steel sheet and variations in alloy concentrations may occur. Moreover, the decarburization may cause the formation of ferrite in the surface layer and a reduction in tensile strength may occur. Therefore, the coiling temperature is preferably 630°C. or lower. The coiling temperature is more preferably 600°C. or lower. No particular limitation is imposed on the lower limit of the coiling temperature. However, to prevent deterioration in cold rollability, the coiling temperature is preferably 500°C. or higher.

The coiled hot-rolled steel sheet may be pickled. No particular limitation is imposed on the pickling conditions.

#### Cold Rolling Step

The cold rolling step is the step of cold-rolling the hot-rolled steel sheet obtained in the hot rolling step. No particular limitation is imposed on the rolling reduction of the cold rolling and its upper limit. However, if the rolling reduction is less than 20%, the microstructure tends to be inhomogeneous. Therefore, the rolling reduction is preferably 20% or more. If the rolling reduction is more than 90%, excessively introduced strains facilitate recrystallization excessively during annealing. In this case, the diameter of prior- $\gamma$  grains may increase, and the strength may deteriorate. Therefore, the rolling reduction is preferably 90% or less. The cold rolling step is not an essential step and may be omitted when the steel microstructure and the mechanical properties satisfy those for aspects of the present invention.

#### Annealing Step

The annealing step is the step of holding the cold-rolled steel sheet or the hot-rolled steel sheet at an annealing temperature equal to or higher than  $A_{C1}$  temperature for 30 seconds or longer, then starting water quenching from a temperature equal to or higher than  $Ms$  temperature to water-cool the resulting steel sheet to 100°C. or lower, and reheating the cooled steel sheet to from 100°C. to 300°C. In a region in which the surface temperature of the steel sheet is equal to or lower than ( $Ms$  temperature+150°C.) during water cooling in the water quenching, the steel sheet is restrained from the front and back sides of the steel sheet using two rolls such that the following conditions (1) to (3) are satisfied, the two rolls being disposed with the steel sheet interposed therebetween:

- (1) the depression amount of each of the two rolls is more than 0 mm and  $t$  mm or less, where  $t$  is the thickness of the steel sheet;
- (2)  $Rn$  and  $rn$  are from 50 mm to 1000 mm, where  $Rn$  and  $rn$  are the roll diameters of the respective two rolls; and
- (3) the inter-roll distance between the two rolls is more than 0 mm and  $(Rn+rn+t)/16$  mm or less.

FIG. 1 shows a schematic illustration of an example of a steel sheet 10 that is restrained by two rolls from the front and back sides of the steel sheet during water cooling in the annealing step such that the above conditions (1) to (3) are satisfied. The two rolls are disposed such that one roll is disposed on the front side of the steel sheet 10 in the cooling water 12 and the other roll is disposed on the back side. The steel sheet 10 is restrained by one roll 11a and the other roll

11b from the front and back sides. In FIG. 1, symbol D1 represents the conveying direction of the steel sheet.

#### Heating to Annealing Temperature Equal to or Higher Than $A_{C1}$ Temperature

If the annealing temperature is lower than the  $A_{C1}$  temperature, austenite is not formed. In this case, it is difficult to obtain a steel sheet containing 20% or more of martensite, and the desired strength is not obtained. Therefore, the annealing temperature is equal to or higher than the  $A_{C1}$  temperature. The annealing temperature is preferably equal to or higher than ( $A_{C1}$  temperature+10°C.). No particular limitation is imposed on the upper limit of the annealing temperature. However, from the viewpoint of optimizing the temperature during water quenching and preventing deterioration in the shape uniformity, the annealing temperature is preferably 900°C. or lower.

The  $A_{C1}$  temperature ( $A_{C1}$  transformation temperature) as used herein is computed using the following formula. In the following formula, (%+symbol of element) means the content (%) by mass of the element.

$$A_{C1}(\text{°C.}) = 723 + 22(\% \text{ Si}) - 18(\% \text{ Mn}) + 17(\% \text{ Cr}) + 4.5(\% \text{ Mo}) + 16(\% \text{ V})$$

#### Holding Time at Annealing Temperature: 30 Seconds or Longer

If the holding time at the annealing temperature is shorter than 30 second, dissolution of carbides and austenite transformation do not proceed sufficiently, and therefore remaining carbides coarsen during subsequent heat treatment. In this case, the dislocation density in the metal phases at the widthwise center of the sheet relative to the dislocation density at the widthwise edges of the sheet decreases, and the shape fixability deteriorates. Moreover, the desired volume fraction of martensite is not obtained, and the desired strength is not obtained. Therefore, the holding time at the annealing temperature is preferably 30 seconds or longer and preferably 35 seconds or longer. No particular limitation is imposed on the upper limit of the holding time at the annealing temperature. However, from the viewpoint of inhibiting an increase in the diameter of austenite grains and preventing deterioration in the shape fixability, the holding time at the annealing temperature is preferably 900 seconds or shorter.

#### Water Quenching Start Temperature: $Ms$ Temperature or Higher

The quenching start temperature is an important factor that determines the volume fraction of martensite, which is a controlling factor of the strength. If the quenching start temperature is lower than  $Ms$  temperature, martensite transformation occurs before quenching, and self-tempering of martensite occurs before quenching. In this case, not only the shape uniformity deteriorates, but also ferrite transformation, pearlite transformation, and bainite transformation occur before quenching. As a result, the volume fraction of martensite decreases and the desired strength is difficult to obtain. Therefore, the water quenching start temperature is equal to or higher than  $Ms$  temperature. The water quenching start temperature is preferably equal to or higher than ( $Ms$  temperature+50°C.). No particular limitation is imposed on the upper limit of the water quenching start temperature, and the water quenching start temperature may be equal to the annealing temperature.

The Ms temperature as used herein is computed using a formula below. In the following formula, (%+symbol of element) means the content (% by mass) of the element, and (% V<sub>M</sub>) is the area fraction (unit: %) of martensite.

$$\text{Ms temperature } (\text{° C.}) = 550 - 350((\% \text{ C.}) / (\% \text{ V}_M)) \\ 100 - 40(\% \text{ Mn}) - 17(\% \text{ Ni}) - 17(\% \text{ Cr}) - 21(\% \text{ Mo})$$

Restraining the steel sheet using the two rolls from the front and back sides of the steel sheet during water cooling in the water quenching is an important factor for obtaining the shape correction effect. Controlling the restraining conditions is an important factor for reducing the variations in the dislocation density in the metal phases over the entire width of the steel sheet. One feature according to aspects of the present invention is that, by restraining the steel sheet to correct the transformation strain generated during water cooling, the shape uniformity of the steel sheet is improved. Therefore, a correction using leveler straightening or skin pass rolling that increases variations in YR and causes deterioration in the shape fixability is unnecessary. Since levelling or skin pass rolling used to correct shape deformation is unnecessary, variations in the dislocation density in the metal phases over the entire width of the steel sheet can be reduced.

The front and back sides as used herein are one surface of the steel sheet and its surface opposite thereto, and any one of them may be used as the front side.

Surface Temperature of Steel Sheet when Steel Sheet is Restrained Using Two Rolls from Front and Back Sides of Steel Sheet (Restraining Temperature): (Ms Temperature+150° C.) or Lower

If the restraining temperature is higher than (Ms temperature+150° C.), martensite transformation occurs after the restraining. In this case, shape deterioration due to transformation expansion by the martensite transformation cannot be prevented, and the shape uniformity deteriorates. Therefore, the restraining temperature is (Ms temperature+150° C.) or lower, preferably (Ms temperature+100° C.) or lower, and more preferably (Ms temperature+50° C.) or lower. No particular limitation is imposed on the lower limit of the restraining temperature, and it is only necessary that the restraining temperature be 0° C. or higher at which water does not freeze.

Depression Amount of Each of Two Rolls: 0 mm or More and t mm or Less, Where t is Thickness of Steel Sheet

FIG. 2 is an enlarged illustration showing a portion near the two rolls in FIG. 1. FIG. 3 is a schematic illustration showing the depression amounts of the rolls. For the convenience of description, only the steel sheet 10 in FIG. 2 is shown in FIG. 3.

As shown in FIGS. 2 and 3, the steel sheet 10 is depressed by the two rolls from the front and back sides. The depression amounts of the rolls as used herein are as follows. The depression amount of a roll in a state in which the roll is in contact with a straight steel sheet with no force applied to the steel sheet is set to 0. The amount (distance) of movement of the roll from the above state toward the steel sheet is used as the depression amount. In FIG. 3, the depression amount of one roll 11a and the depression amount of the other roll 11b are shown with respective symbols B1 and B2 assigned thereto.

In accordance with aspects of the present invention, the depression amount of each of the two rolls is more than 0 mm and t mm or less, where t is the thickness of the steel sheet. If the depression amount is less than 0 mm, the rolls are not in contact with the steel sheet. If the depression

amount is 0 mm, although the rolls are in contact with the steel sheet, the steel sheet is not depressed by the rolls. To obtain the shape correction effect, the depression amount must be more than 0 mm. The depression amount is preferably 0.1 mm or more. To obtain the shape correction effect, it is necessary to increase the depression amount. However, if the depression amount is more than t mm, a bending force is applied to the steel sheet, and strain tends to be generated in the steel sheet, particularly in the widthwise central portion of the sheet. In this case, the ratio of the dislocation density in the metal phases at the widthwise edges of the sheet to the dislocation density at the widthwise center of the sheet is less than 100%, and the shape fixability deteriorates. Therefore, the depression amount is t mm or less. The depression amount is preferably (t-0.1 mm) or less.

No particular limitation is imposed on the barrel length of each of the two rolls so long as the depression amount is in the above range. However, to restrain the steel sheet by the two rolls stably from the front and back sides of the steel sheet, it is preferable that the barrel length of each of the two rolls is longer than the width of the steel sheet.

Rn and rn: from 50 mm to 1000 mm, Where Rn and rn Are Roll Diameters of Respective Two Rolls

The area of contact between a roll and the steel sheet varies depending on the diameter of the roll. The larger the roll diameter, the higher the shape correction ability. To increase the shape correction ability to obtain the desired shape uniformity, the roll diameter must be 50 mm or more. The roll diameter is preferably 70 mm or more and more preferably 100 mm or more. A cooling nozzle cannot be disposed near the rolls. Therefore, if the roll diameter is excessively large, the cooling capacity near the rolls is low and the shape uniformity deteriorates. To obtain the cooling capacity that allows the desired shape uniformity, the roll diameter must be 1000 mm or less. The roll diameter is preferably 700 mm or less and more preferably 500 mm or less. The roll diameters of the two rolls may differ from each other so long as the desired shape uniformity is obtained.

Inter-Roll Distance Between Two Rolls: More Than 0 mm and (Rn+rn+t)/16 mm or Less

The inter-roll distance between the two rolls in accordance with aspects of the present invention is the center-to-center distance between the two rolls in the conveying direction (rolling direction) of the steel sheet. Let the center of the one roll 11a be C1, and the center of the other roll 11b be C2, as shown in FIG. 2. Then the distance between the center C1 and the center C2 in the conveying direction D1 of the steel sheet is the inter-roll distance A1.

More particularly, the inter-roll distance A1 is determined as A0·cos X, where A0 is the length of a line segment connecting the center C1 and the center C2 such that the length is shortest, and X is the angle between the line segment and the conveying direction D1.

If the two rolls sandwiching the steel sheet 10 therebetween are disposed such that the center C1 of the one roll 11a and the center C2 of the other roll 11b are located perpendicular to the steel sheet 10, the inter-roll distance is 0 mm, as shown in FIG. 4.

When the inter-roll distance is large, it is necessary to increase the depression amount in order to obtain the shape correction effect. However, if the depression amount is increased, a bending force is applied to the steel sheet. Therefore, strain tends to be generated in the steel sheet, particularly in the widthwise central portion of the sheet. In this case, the ratio of the dislocation density in the metal phases at the widthwise edges of the sheet to the dislocation density at the widthwise center of the sheet is less than

100%, and the shape fixability deteriorates. Therefore, the inter-roll distance is  $(Rn+rn+t)/16$  mm or less. The inter-roll distance is preferably  $(Rn+rn+t)/18$  mm or less. To obtain the shape correction effect, the inter-roll distance must be more than 0 mm.

The number of rolls may be three or more so long as sufficient cooling capacity can be obtained and the desired shape uniformity and the desired shape fixability can be obtained. When the number of rolls is three or more, it is only necessary that the inter-roll distance between two rolls among the three or more rolls that are adjacent to each other in the rolling direction (longitudinal direction) of the steel sheet be more than 0 mm and  $(Rn+rn+t)/16$  mm or less.

Water Cooling to 100° C. or Lower

If the temperature after water cooling is higher than 100° C., martensite transformation proceeds after the water cooling to the extent that the shape uniformity is adversely affected. Therefore, the temperature of the steel sheet after exit from the water bath must be 100° C. or lower and is preferably 80° C. or lower.

Reheating to from 100° C. to 300° C.

After the water cooling, the steel sheet is reheated to temper the martensite formed during the water cooling, and the strain introduced in the martensite can thereby be removed. As a result, the amount of strain is constant over the entire width of the steel sheet, and the variations in the dislocation density in the metal phases can be reduced, and the shape fixability can be improved. If the reheating temperature is lower than 100° C., the above effect is not obtained. Therefore, the reheating temperature is 100° C. or higher. The reheating temperature is preferably 130° C. or higher. If the steel sheet is tempered at higher than 300° C., transformation shrinkage due to tempering causes deterioration in the shape uniformity. Therefore, the reheating temperature is 300° C. or lower. The reheating temperature is preferably 260° C. or lower.

The hot-rolled steel sheet subjected to the hot rolling step may be subjected to heat treatment for softening the micro-structure or may be subjected to temper rolling after the annealing step in order to adjust the shape. Moreover, the surface of the steel sheet may be plated with Zn, Al, etc.

Next, a member according to aspects of the present invention and a method for producing the member will be described.

A member according to aspects of the present invention is prepared by subjecting the steel sheet according to aspects of the present invention to at least one of forming and welding. The method for producing the member according to aspects of the present invention includes the step of subjecting the steel sheet produced by the steel sheet production method according to aspects of the present invention to at least one of forming and welding.

Since the steel sheet according to aspects of the present invention has high strength, excellent shape uniformity, and excellent shape fixability, the member obtained using the steel sheet according to aspects of the present invention has high strength and high dimensional accuracy. Therefore, the member according to aspects of the present invention can be preferably used, for example, for components required to have high strength and high dimensional accuracy. The member according to aspects of the present invention can be preferably used, for example, for automotive parts.

A general processing method such as press working can be used for the forming without any limitation. A general welding method such as spot welding or arc welding can be used for the welding.

## EXAMPLES

Aspects of the present invention will be described specifically with reference to Examples.

### Example 1

A 1.4 mm thick cold-rolled steel sheet obtained by cold rolling under conditions shown in Table 1 was annealed under conditions shown in Table 1 to thereby produce a steel sheet having properties described in Table 2. The temperature of the steel sheet when it passed between the restraining rolls was measured using a contact-type thermometer attached to one of the rolls. The two rolls were disposed such that the depression amounts of the two rolls were the same.

In the hot rolling before the cold rolling, the slab heating temperature of the steel slab was set to 1250° C., and the slab soaking time during the slab heating was set to 60 minutes. The finish rolling temperature was set to 880° C., and the cooling temperature was set to 550° C.

The  $A_{C1}$  temperature of each steel sheet used was 706° C., and its  $M_s$  temperature was 410° C.

TABLE 1

| No. | %  | Cold              |                 | Annealing conditions  |           |         |                 |      |     |    |
|-----|----|-------------------|-----------------|-----------------------|-----------|---------|-----------------|------|-----|----|
|     |    | Rolling reduction | Sheet thickness | Annealing temperature | Annealing |         | Quenching start | *1   | *2  |    |
|     |    |                   |                 |                       | holding   | time    |                 |      |     |    |
|     |    | No.               | %               | mm                    | ° C.      | Seconds | ° C.            | ° C. | mm  | mm |
| 1   | 56 | 1                 | 56              | 1.4                   | 860       | 60      | 775             | 300  | 0.5 | 5  |
| 2   | 56 | 2                 | 56              | 1.4                   | 860       | 60      | 782             | —    | —   | —  |
| 3   | 56 | 3                 | 56              | 1.4                   | 860       | 60      | 766             | 310  | 0.5 | 15 |
| 4   | 56 | 4                 | 56              | 1.4                   | 860       | 60      | 769             | 305  | 0.5 | 10 |
| 5   | 56 | 5                 | 56              | 1.4                   | 860       | 60      | 760             | 300  | 1.6 | 30 |
| 6   | 56 | 6                 | 56              | 1.4                   | 860       | 60      | 776             | 300  | 1.2 | 20 |
| 7   | 56 | 7                 | 56              | 1.4                   | 860       | 60      | 777             | 320  | 0.5 | 50 |
| 8   | 56 | 8                 | 56              | 1.4                   | 860       | 60      | 780             | 320  | 0.5 | 5  |

TABLE 1-continued

| No. | Annealing conditions      |                           |                                        |                               |                     |
|-----|---------------------------|---------------------------|----------------------------------------|-------------------------------|---------------------|
|     | Roll diameter<br>Rn<br>mm | Roll diameter<br>rn<br>mm | Water cooling stop temperature<br>° C. | Reheating temperature<br>° C. | Remarks             |
| 1   | 300                       | 300                       | 50                                     | 150                           | Inventive Example   |
| 2   | —                         | —                         | 50                                     | 150                           | Comparative Example |
| 3   | 600                       | 300                       | 50                                     | 150                           | Inventive Example   |
| 4   | 300                       | 500                       | 50                                     | 150                           | Inventive Example   |
| 5   | 300                       | 300                       | 50                                     | 150                           | Comparative Example |
| 6   | 300                       | 300                       | 50                                     | 120                           | Inventive Example   |
| 7   | 300                       | 300                       | 50                                     | 150                           | Comparative Example |
| 8   | 300                       | 300                       | 50                                     | 70                            | Comparative Example |

\*1: The surface temperature of the steel sheet when it was restrained by the rolls.

\*2: The depression amount of each of the two rolls.

\*3: The inter-roll distance between the two rolls.

## 2. Evaluation Methods

For each of the steel sheets obtained under various production conditions, the steel microstructure was analyzed to examine microstructure fractions, and a tensile test was performed to evaluate tensile properties such as tensile strength. Moreover, the warpage of the steel sheet was used to evaluate the shape uniformity, and X-ray diffraction measurement was performed to examine the dislocation density in the metal phases. The evaluation methods are as follows.

### (Area Fraction of Martensite)

A test sample was taken from each steel sheet so as to extend in the rolling direction of the steel sheet and a direction perpendicular to the rolling direction, and a cross section along the sheet thickness L and parallel to the rolling direction was polished to a mirror finish and etched with a nital solution to cause the microstructure to appear. The sample with the microstructure appearing therein was observed using a scanning electron microscope. A  $16 \times 15$  lattice with a spacing of  $4.8 \mu\text{m}$  was placed on a region with actual lengths of  $82 \mu\text{m} \times 57 \mu\text{m}$  in an SEM image at a magnification of  $1500\times$ , and the area fraction of martensite was examined using a point counting method in which the number of points on each phase was counted. The area fraction was the average of three area fractions determined in different SEM images at a magnifications of  $1500\times$ . The measurement was performed at a depth of one-fourth the sheet thickness. Martensite is a white microstructure, and tempered martensite includes fine carbides precipitated therein. Ferrite is a black microstructure. Depending on the plane orientations of block grains and the degree of etching, internal carbides may be less likely to appear. In such a case, it is necessary to perform etching sufficiently to check the internal carbides.

The area fraction of the metal phases other than ferrite and martensite was computed by subtracting the total area fraction of ferrite and martensite from 100%.

### (Tensile Test)

JIS No. 5 test specimens having a gauge length of 50 mm and a gauge width of 25 mm and extending in the rolling direction were taken from different widthwise positions from the widthwise central portion of each steel sheet, and a tensile test was performed at a strain rate of 10 mm/minute according to JIS 22241 (2011) to thereby measure tensile strength (TS), yield strength (YS), and variations in yield ratio ( $\Delta\text{YR}$ ). The YR was computed using  $\text{YS}/\text{TS} \times 100$ . The TS and YS are the TS and YS at the widthwise center of the

sheet. The  $\Delta\text{YR}$  is the difference between the YR at the widthwise center of the sheet and the YR at a widthwise edge of the sheet.

### (Evaluation of Shape Uniformity of Steel Sheet)

Each steel sheet was sheared to a length of 1 m in the longitudinal direction (rolling direction) of the steel sheet while the original width of the steel sheet was maintained, and the sheared steel sheet was placed on a horizontal table. The sheared steel sheet was placed on the horizontal table such that the horizontal table and the steel sheet were in contact with each other at as many contact points as possible (at two or more points). The amount of warpage was determined by lowering a horizontal plate from a position higher than the steel sheet until the horizontal plate came into contact with the steel sheet and subtracting the thickness of the steel sheet from the distance between the horizontal table and the horizontal plate at the contact position at which the horizontal plate was in contact with the steel sheet. The above distance is the distance in a direction perpendicular to a horizontal surface of the horizontal table (the vertical direction). After the measurement of the amount of warpage with one surface of the steel sheet facing upward, the amount of warpage was measured with the other surface facing upward, and the largest one of the measured warpage amounts was used as the maximum amount of warpage. When the steel sheet was sheared in the longitudinal direction, the clearance between the cutting edges of the shearing machine was set to 4% (the upper limit of the control range is 10%).

### (Measurement of Dislocation Density in Metal Phases)

For each of the steel sheets, the dislocation density in the metal phases was measured by methods described below. Specifically, on the surface of the steel sheet, the ratio of the dislocation density in the metal phases at a widthwise edge of the sheet to the dislocation density in the metal phases at the widthwise center of the sheet was computed. Moreover, at the thicknesswise center of the sheet, the ratio of the dislocation density in the metal phases at the widthwise edge of the sheet to the dislocation density in the metal phases at the widthwise center of the sheet was computed.

First, the method for computing the ratio of the dislocation density in the metal phases at the widthwise edge of the sheet to the dislocation density in the metal phases at the widthwise center of the sheet on the surface of the steel sheet will be described.

Samples having a width of 10 mm  $\times$  a conveying direction length of 10 mm were taken from a widthwise central

portion of each steel sheet and a widthwise edge portion of the steel sheet (an outermost edge portion of the steel sheet). The surface of each steel sheet sample was polished to remove scales, and the polished surface of the steel sheet was subjected to X-ray diffraction measurement. The amount of the steel sheet polished to remove scales was less than 1  $\mu\text{m}$ . The radiation source was Co. Since the analysis depth of Co is about 20  $\mu\text{m}$ , the dislocation density in the metal phases on the surface of the steel sheet is the dislocation density in the metal phases in the range of 0 to 20  $\mu\text{m}$  from the surface of the steel sheet. The dislocation density in the metal phases was determined using a method in which the dislocation density was converted from a strain determined from the half width  $\beta$  in the X-ray diffraction measurement. To extract the strain, the Williamson-Hall method described below was used. The half width is influenced by the size  $D$  of crystallites and the strain  $\epsilon$  and can be computed as the sum of these factors using the following formula.

$$\beta = \beta_1 + \beta_2 = (0.9\lambda/(D \times \cos \theta)) + 2\epsilon \times \tan \theta$$

By modifying this formula,  $\beta \cos \theta/\lambda = 0.9\lambda/D + 2\epsilon \times \sin \theta/\lambda$  is obtained.  $\beta \cos \theta/\lambda$  was plotted versus  $\sin \theta/\lambda$ , and the strain  $\epsilon$  was computed from the gradient of the straight line. The diffraction lines used for the computation were (110), (211), and (220). To convert the strain  $\epsilon$  to the dislocation density in the metal phases,  $\rho = 14.4\epsilon^2/b^2$  was used. Here,  $\theta$  is a peak angle computed using the  $\theta-2\theta$  method for X-ray

to remove scales. The amount of the steel sheet polished to remove scales was less than 1  $\mu\text{m}$ . Next, the surface of each sample was ground to the thicknesswise center of the sheet, and the resulting sample was subjected to X-ray diffraction measurement using the same method as that for the measurement on the surface of the steel sheet. Since the analysis depth of Co is about 20  $\mu\text{m}$ , the dislocation density in the metal phases at the thicknesswise center of the sheet is the dislocation density in the metal phases in the range of 0 to 20  $\mu\text{m}$  from the center of the steel sheet. Based on the results of the measurement, the ratio of the dislocation density in the metal phases on the surface of the widthwise edge of the sheet to the dislocation density in the metal phases on the surface of the widthwise center of the sheet was determined.

In the thickness direction of the sheet, the dislocation density in the metal phases tends to be largest in the thicknesswise central portion of the sheet and tends to be smallest on the surface. Therefore, in the present Example, the dislocation density in the metal phases was measured on the surface and at the thicknesswise central portion of the sheet, and the measured dislocation densities were used to define the dislocation density ratios in the metal phases in the width direction at all thicknesswise positions of the sheet.

### 3. Evaluation Results

The results of the evaluation are shown in Table 2.

TABLE 2

| No. | Microstructure |        |             |         | Tensile properties |           |           |          | Shape         |                     |
|-----|----------------|--------|-------------|---------|--------------------|-----------|-----------|----------|---------------|---------------------|
|     | M<br>%         | F<br>% | Others<br>% | *1<br>% | *2<br>%            | YS<br>MPa | TS<br>MPa | AYR<br>% | warpage<br>mm | Maximum             |
| 1   | 97             | 2      | 1           | 128     | 122                | 1257      | 1522      | 0        | 2             | Inventive Example   |
| 2   | 96             | 2      | 2           | 95      | 99                 | 1251      | 1517      | 6        | 22            | Comparative Example |
| 3   | 97             | 2      | 1           | 117     | 122                | 1257      | 1522      | -2       | 5             | Inventive Example   |
| 4   | 97             | 1      | 2           | 124     | 122                | 1257      | 1512      | -1       | 3             | Inventive Example   |
| 5   | 98             | 1      | 1           | 94      | 119                | 1239      | 1541      | 4        | 4             | Comparative Example |
| 6   | 97             | 1      | 2           | 108     | 132                | 1287      | 1532      | -3       | 3             | Inventive Example   |
| 7   | 99             | 1      | 0           | 98      | 110                | 1267      | 1522      | 4        | 5             | Comparative Example |
| 8   | 98             | 1      | 1           | 142     | 143                | 1396      | 1581      | -5       | 5             | Comparative Example |

M: Area fraction of martensite,

F: Area fraction of ferrite,

Others: Area fraction of other metal phases

\*1: The ratio of the dislocation density in the metal phases at the widthwise edge of the sheet to the dislocation density in the metal phases at the widthwise center of the sheet on the surface of the steel sheet (the dislocation density on the surface of the widthwise edge of the sheet/the dislocation density on the surface of the widthwise center of the sheet).

\*2: The ratio of the dislocation density in the metal phases at the widthwise center of the sheet at the thicknesswise central portion of the sheet to the dislocation density in the metal phases at the widthwise edge of the sheet at the thicknesswise central portion of the sheet (the dislocation density in the thicknesswise central portion of the sheet/the dislocation density in the thicknesswise central portion at the widthwise center of the sheet).

50

diffraction, and  $\lambda$  is the wavelength of the X-ray used for the X-ray diffraction.  $b$  is the Burgers vector of  $\text{Fe}(\alpha)$  and is 0.25 nm in the present Example. Then the ratio of the dislocation density in the metal phases on the surface of the widthwise edge of the sheet to the dislocation density in the metal phases on the surface of the widthwise center of the sheet on the surface of the steel sheet was determined.

Next, the method for computing the ratio of the dislocation density in the metal phases at the widthwise edge of the sheet to the dislocation density in the metal phases at the widthwise center of the sheet will be described.

Samples with a width of 20 mm and a conveying direction length of 20 mm was taken from a widthwise central portion of each steel sheet and a widthwise edge portion of the steel sheet. The surface of each steel sheet sample was polished

to remove scales. The amount of the steel sheet polished to remove scales was less than 1  $\mu\text{m}$ . Next, the surface of each sample was ground to the thicknesswise center of the sheet, and the resulting sample was subjected to X-ray diffraction measurement using the same method as that for the measurement on the surface of the steel sheet. Since the analysis depth of Co is about 20  $\mu\text{m}$ , the dislocation density in the metal phases at the thicknesswise center of the sheet is the dislocation density in the metal phases in the range of 0 to 20  $\mu\text{m}$  from the center of the steel sheet. Based on the results of the measurement, the ratio of the dislocation density in the metal phases on the surface of the widthwise edge of the sheet to the dislocation density in the metal phases on the surface of the widthwise center of the sheet was determined.

In the thickness direction of the sheet, the dislocation density in the metal phases tends to be largest in the thicknesswise central portion of the sheet and tends to be smallest on the surface. Therefore, in the present Example, the dislocation density in the metal phases was measured on the surface and at the thicknesswise central portion of the sheet, and the measured dislocation densities were used to define the dislocation density ratios in the metal phases in the width direction at all thicknesswise positions of the sheet.

60

**Example 2**

1. Production of Steel Sheets for Evaluation

Steel having a chemical composition shown in Table 3 with the balance being Fe and incidental impurities was obtained by steel making using a vacuum melting furnace and caged to obtain a caged product having a thickness of 27 mm. The caged product obtained was hot-rolled. Then

samples to be cold-rolled were obtained by grinding the hot-rolled steel sheet. These samples were cold-rolled at a rolling reduction shown in Table 4 or 5 to thereby produce cold-rolled steel sheets having a thickness shown in Table 4 or 5. Some samples obtained by grinding the hot-rolled steel sheet were not subjected to cold rolling. In the tables, a sample with “-” in the rolling reduction column was not subjected to cold rolling. Next, the above-obtained hot-rolled steel sheets and the cold-rolled steel sheets were annealed under conditions shown in Tables 4 or 5 to thereby produce steel sheets. Each blank in Table 3 means that a corresponding element was not added intentionally. This

means not only that the element was not added (0% by mass) but also that the element was inevitably contained. The temperature of the steel sheet when it passed between the restraining rolls was measured using a contact-type thermometer attached to one of the rolls. The two rolls were disposed such that the depression amounts of the two rolls were the same.

In the hot rolling before the cold rolling, the slab heating temperature of the steel slab was set to 1250° C., and the slab 10 soaking time during slab heating was set to 60 minutes. The finish rolling temperature was set to 880° C., and the cooling temperature was set to 550° C.

TABLE 3

| Steel | Chemical composition (% by mass) |      |      |       |        |       |        |        |       |       |    |    |    | $A_{c1}$<br>temperature |       |       |       |        |
|-------|----------------------------------|------|------|-------|--------|-------|--------|--------|-------|-------|----|----|----|-------------------------|-------|-------|-------|--------|
| type  | C                                | Si   | Mn   | P     | S      | Al    | N      | B      | Nb    | Ti    | Cu | Ni | Cr | Mo                      | V     | Sb    | Sn    | (° C.) |
| A     | 0.06                             | 1.00 | 2.20 | 0.007 | 0.0008 | 0.051 | 0.0021 |        |       |       |    |    |    |                         |       |       |       | 705    |
| B     | 0.11                             | 0.90 | 0.20 | 0.008 | 0.0003 | 0.068 | 0.0048 |        |       |       |    |    |    |                         |       |       |       | 739    |
| C     | 0.14                             | 1.40 | 2.40 | 0.008 | 0.0005 | 0.080 | 0.0021 |        |       |       |    |    |    |                         |       |       |       | 711    |
| D     | 0.22                             | 0.40 | 1.50 | 0.018 | 0.0002 | 0.021 | 0.0043 |        |       |       |    |    |    |                         |       |       |       | 705    |
| E     | 0.26                             | 0.20 | 1.00 | 0.010 | 0.0010 | 0.008 | 0.0043 |        |       |       |    |    |    |                         |       |       |       | 709    |
| F     | 0.28                             | 1.40 | 1.50 | 0.010 | 0.0010 | 0.049 | 0.0058 |        |       |       |    |    |    |                         |       |       |       | 727    |
| G     | 0.22                             | 1.50 | 2.80 | 0.007 | 0.0040 | 0.036 | 0.0014 |        |       |       |    |    |    |                         |       |       |       | 706    |
| H     | 0.42                             | 1.40 | 0.80 | 0.007 | 0.0010 | 0.078 | 0.0034 |        |       |       |    |    |    |                         |       |       |       | 739    |
| I     | 0.54                             | 0.12 | 0.25 | 0.006 | 0.0007 | 0.096 | 0.0046 |        |       |       |    |    |    |                         |       |       |       | 721    |
| J     | 0.28                             | 1.60 | 1.40 | 0.025 | 0.0002 | 0.092 | 0.0028 |        |       |       |    |    |    |                         |       |       |       | 733    |
| K     | 0.27                             | 1.80 | 1.60 | 0.009 | 0.0009 | 0.026 | 0.0031 |        |       |       |    |    |    |                         |       |       |       | 734    |
| L     | 0.15                             | 0.01 | 2.90 | 0.016 | 0.0004 | 0.039 | 0.0028 |        |       |       |    |    |    |                         |       |       |       | 671    |
| M     | 0.14                             | 0.07 | 3.10 | 0.005 | 0.0004 | 0.050 | 0.0015 |        |       |       |    |    |    |                         |       |       |       | 669    |
| N     | 0.26                             | 0.90 | 1.50 | 0.006 | 0.0010 | 0.066 | 0.0053 |        |       |       |    |    |    |                         | 0.05  |       |       | 717    |
| O     | 0.24                             | 0.80 | 1.70 | 0.038 | 0.0006 | 0.051 | 0.0040 | 0.0100 |       |       |    |    |    |                         | 0.04  |       |       | 710    |
| P     | 0.28                             | 0.40 | 0.90 | 0.006 | 0.0020 | 0.062 | 0.0027 |        |       |       |    |    |    |                         | 0.04  | 0.08  | 0.005 | 717    |
| Q     | 0.32                             | 0.05 | 0.60 | 0.009 | 0.0002 | 0.063 | 0.0088 | 0.0060 | 0.004 |       |    |    |    |                         |       |       |       | 713    |
| R     | 0.15                             | 1.20 | 2.40 | 0.007 | 0.0004 | 0.038 | 0.0051 |        |       |       |    |    |    |                         | 0.005 | 0.004 |       | 706    |
| S     | 0.18                             | 1.40 | 2.30 | 0.006 | 0.0003 | 0.040 | 0.0037 | 0.0007 |       |       |    |    |    |                         |       |       |       | 712    |
| T     | 0.24                             | 1.30 | 2.10 | 0.017 | 0.0005 | 0.034 | 0.0019 |        |       |       |    |    |    |                         | 0.008 | 0.005 |       | 714    |
| U     | 0.63                             | 1.10 | 1.20 | 0.019 | 0.0002 | 0.035 | 0.0021 |        |       |       |    |    |    |                         |       |       |       | 726    |
| V     | 0.04                             | 1.20 | 1.20 | 0.006 | 0.0002 | 0.077 | 0.0055 |        |       |       |    |    |    |                         |       |       |       | 728    |
| W     | 0.21                             | 2.40 | 1.05 | 0.008 | 0.0010 | 0.023 | 0.0028 |        |       |       |    |    |    |                         |       |       |       | 757    |
| X     | 0.22                             | 0.12 | 3.40 | 0.026 | 0.0006 | 0.069 | 0.0024 |        |       |       |    |    |    |                         |       |       |       | 664    |
| Y     | 0.22                             | 0.16 | 0.04 | 0.008 | 0.0007 | 0.059 | 0.0010 |        |       |       |    |    |    |                         |       |       |       | 726    |
| Z     | 0.28                             | 0.84 | 1.20 | 0.070 | 0.0004 | 0.069 | 0.0058 |        |       |       |    |    |    |                         |       |       |       | 720    |
| AA    | 0.26                             | 0.07 | 1.32 | 0.007 | 0.0080 | 0.059 | 0.0028 |        |       |       |    |    |    |                         |       |       |       | 701    |
| AB    | 0.25                             | 0.11 | 1.31 | 0.006 | 0.0003 | 0.150 | 0.0021 |        |       |       |    |    |    |                         |       |       |       | 702    |
| AC    | 0.21                             | 0.05 | 1.28 | 0.018 | 0.0008 | 0.071 | 0.0150 |        |       |       |    |    |    |                         |       |       |       | 701    |
| AD    | 0.20                             | 0.40 | 1.40 | 0.012 | 0.0007 | 0.035 | 0.0040 | 0.0080 |       | 0.080 |    |    |    |                         |       |       |       | 707    |
| AE    | 0.20                             | 0.20 | 1.60 | 0.012 | 0.0009 | 0.045 | 0.0050 |        |       | 0.050 |    |    |    |                         | 0.08  | 0.05  |       | 700    |
| AF    | 0.21                             | 0.40 | 1.40 | 0.010 | 0.0007 | 0.045 | 0.0050 | 0.0100 |       | 0.060 |    |    |    |                         | 0.12  |       |       | 707    |
| AG    | 0.20                             | 0.60 | 1.20 | 0.012 | 0.0007 | 0.030 | 0.0040 | 0.0012 |       | 0.080 |    |    |    |                         | 0.12  |       |       | 717    |
| AH    | 0.20                             | 0.40 | 1.40 | 0.012 | 0.0005 | 0.045 | 0.0050 | 0.0016 | 0.015 |       |    |    |    |                         |       |       |       | 707    |
| AI    | 0.19                             | 0.50 | 1.80 | 0.014 | 0.0007 | 0.045 | 0.0050 |        |       | 0.05  |    |    |    |                         | 0.008 |       |       | 702    |
| AJ    | 0.20                             | 0.30 | 1.40 | 0.012 | 0.0007 | 0.040 | 0.0050 | 0.0010 | 0.012 |       |    |    |    |                         | 0.020 |       |       | 704    |
| AK    | 0.20                             | 0.40 | 1.50 | 0.012 | 0.0007 | 0.045 | 0.0050 | 0.0015 |       | 0.120 |    |    |    |                         | 0.06  | 0.012 |       | 706    |

TABLE 4

| No. | Steel<br>type | Sheet<br>thickness<br>mm | rolling<br>Reduction<br>% | Annealing<br>temperature<br>° C. | Annealing<br>holding<br>time<br>Seconds | Quenching<br>start<br>temperature<br>° C. | Annealing conditions |          |          |
|-----|---------------|--------------------------|---------------------------|----------------------------------|-----------------------------------------|-------------------------------------------|----------------------|----------|----------|
|     |               |                          |                           |                                  |                                         |                                           | *1<br>° C.           | *2<br>mm | *3<br>mm |
| 1   | A             | 1.4                      | 56                        | 760                              | 60                                      | 831                                       | 300                  | 0.5      | 5        |
| 2   |               | 1.4                      | 56                        | 760                              | 60                                      | 801                                       | 300                  | 0.5      | 10       |
| 3   |               | 1.4                      | 56                        | 760                              | 60                                      | 709                                       | —                    | —        | —        |
| 4   |               | 1.4                      | 56                        | 760                              | 60                                      | 845                                       | 300                  | 0.5      | 30       |
| 5   | B             | 1.4                      | 56                        | 800                              | 60                                      | 717                                       | 300                  | 0.5      | 30       |
| 6   |               | 1.4                      | 56                        | 800                              | 60                                      | 900                                       | 300                  | 0.2      | 30       |
| 7   |               | 1.4                      | 56                        | 800                              | 60                                      | 887                                       | 300                  | 0.8      | 30       |
| 8   |               | 1.4                      | 56                        | 800                              | 60                                      | 761                                       | 300                  | 1.4      | 30       |
| 9   | C             | 1.4                      | 56                        | 820                              | 60                                      | 830                                       | 300                  | 0.5      | 20       |

TABLE 4-continued

|    |     |     |     |     |     |     |     |     |
|----|-----|-----|-----|-----|-----|-----|-----|-----|
| 10 | 1.4 | 56  | 820 | 60  | 858 | 300 | 0.5 | 15  |
| 11 | 1.4 | 56  | 820 | 60  | 894 | 300 | 0.5 | 30  |
| 12 | 1.4 | 56  | 820 | 60  | 767 | 300 | 0.5 | 30  |
| 13 | D   | 1.4 | 56  | 872 | 60  | 827 | 300 | 0.5 |
| 14 |     | 1.4 | 56  | 880 | 60  | 819 | 300 | 0.5 |
| 15 |     | 1.4 | 56  | 884 | 60  | 779 | 300 | 0.5 |
| 16 |     | 1.4 | 56  | 898 | 60  | 803 | 300 | 0.5 |
| 17 |     | 1.4 | 56  | 867 | 60  | 731 | 300 | 0.5 |
| 18 | 1.4 | 56  | 883 | 60  | 860 | 300 | 0.1 | 30  |
| 19 | 1.4 | 56  | 899 | 60  | 714 | 300 | 1.2 | 30  |
| 20 | 1.4 | 56  | 888 | 60  | 738 | 300 | 1.6 | 30  |
| 21 | F   | 1.4 | 56  | 894 | 60  | 806 | 550 | 0.5 |
| 22 |     | 1.4 | 56  | 882 | 60  | 835 | 400 | 0.5 |
| 23 |     | 1.4 | 56  | 882 | 60  | 835 | 300 | 0.5 |
| 24 |     | 1.4 | 56  | 890 | 60  | 830 | 150 | 0.5 |
| 25 | G   | 1.4 | 56  | 895 | 60  | 807 | 520 | 0.5 |
| 26 |     | 1.4 | 56  | 885 | 60  | 763 | 410 | 0.5 |
| 27 |     | 1.4 | 56  | 885 | 60  | 763 | 150 | 0.5 |
| 28 |     | 1.4 | 56  | 882 | 60  | 758 | 50  | 0.5 |
| 29 | H   | 3.2 | —   | 815 | 60  | 733 | 300 | 0.5 |
| 30 |     | 1.9 | 40  | 850 | 60  | 772 | 300 | 0.5 |
| 31 | 0.6 | 80  | 870 | 60  | 829 | 300 | 0.5 | 15  |
| 32 | I   | 1.4 | 56  | 770 | 60  | 741 | 200 | 0.5 |
| 33 | J   | 1.4 | 56  | 890 | 60  | 730 | 300 | 0.5 |
| 34 | 1.4 | 56  | 880 | 20  | 799 | 300 | 0.5 | 15  |
| 35 | 1.4 | 56  | 889 | 360 | 767 | 300 | 0.5 | 15  |
| 36 | K   | 1.4 | 56  | 879 | 40  | 755 | 300 | 0.5 |
| 37 |     | 1.4 | 56  | 886 | 60  | 550 | 300 | 0.5 |
| 38 |     | 1.4 | 56  | 870 | 60  | 350 | 300 | 0.5 |
| 39 | L   | 1.4 | 56  | 863 | 60  | 650 | 300 | 0.5 |
| 40 | 1.4 | 56  | 861 | 60  | 340 | 300 | 0.5 | 15  |
| 41 | 1.4 | 56  | 873 | 60  | 450 | 300 | 0.5 | 15  |
| 42 | M   | 1.4 | 56  | 891 | 60  | 702 | 300 | 0.5 |
| 43 |     | 1.4 | 56  | 875 | 60  | 727 | 300 | 0.5 |
| 44 | 1.4 | 56  | 878 | 60  | 635 | 300 | 0.5 | 15  |

## Annealing conditions

| No. | Roll diameter<br>Rn<br>mm | Roll diameter<br>rn<br>mm | Watercooling<br>stop<br>temperature<br>° C. | Reheating<br>temperature<br>° C. | Remarks             |
|-----|---------------------------|---------------------------|---------------------------------------------|----------------------------------|---------------------|
| 1   | 300                       | 300                       | 50                                          | 150                              | Inventive Example   |
| 2   | 300                       | 300                       | 50                                          | 150                              | Inventive Example   |
| 3   | —                         | —                         | 50                                          | 150                              | Comparative Example |
| 4   | 300                       | 300                       | 50                                          | 150                              | Inventive Example   |
| 5   | 300                       | 300                       | 50                                          | 150                              | Inventive Example   |
| 6   | 300                       | 300                       | 50                                          | 150                              | Inventive Example   |
| 7   | 300                       | 300                       | 50                                          | 150                              | Inventive Example   |
| 8   | 300                       | 300                       | 50                                          | 150                              | Inventive Example   |
| 9   | 40                        | 300                       | 50                                          | 150                              | Comparative Example |
| 10  | 70                        | 200                       | 50                                          | 150                              | Inventive Example   |
| 11  | 400                       | 300                       | 50                                          | 150                              | Inventive Example   |
| 12  | 300                       | 500                       | 50                                          | 150                              | Inventive Example   |
| 13  | 300                       | 300                       | 50                                          | 150                              | Inventive Example   |
| 14  | 300                       | 300                       | 50                                          | 150                              | Inventive Example   |
| 15  | 300                       | 300                       | 50                                          | 150                              | Inventive Example   |
| 16  | 300                       | 300                       | 50                                          | 150                              | Comparative Example |
| 17  | 300                       | 300                       | 50                                          | 150                              | Inventive Example   |
| 18  | 300                       | 300                       | 50                                          | 150                              | Inventive Example   |
| 19  | 300                       | 300                       | 50                                          | 150                              | Inventive Example   |
| 20  | 300                       | 300                       | 50                                          | 150                              | Comparative Example |
| 21  | 150                       | 150                       | 50                                          | 150                              | Comparative Example |
| 22  | 150                       | 150                       | 50                                          | 150                              | Inventive Example   |
| 23  | 150                       | 150                       | 50                                          | 150                              | Inventive Example   |
| 24  | 150                       | 150                       | 50                                          | 150                              | Inventive Example   |
| 25  | 150                       | 150                       | 50                                          | 150                              | Comparative Example |
| 26  | 150                       | 150                       | 50                                          | 150                              | Inventive Example   |
| 27  | 150                       | 150                       | 50                                          | 150                              | Inventive Example   |
| 28  | 150                       | 150                       | 50                                          | 150                              | Inventive Example   |
| 29  | 150                       | 150                       | 50                                          | 150                              | Inventive Example   |
| 30  | 150                       | 150                       | 50                                          | 150                              | Inventive Example   |
| 31  | 150                       | 150                       | 50                                          | 150                              | Inventive Example   |
| 32  | 150                       | 150                       | 50                                          | 150                              | Inventive Example   |
| 33  | 150                       | 150                       | 50                                          | 150                              | Inventive Example   |
| 34  | 150                       | 150                       | 50                                          | 150                              | Comparative Example |
| 35  | 150                       | 150                       | 50                                          | 150                              | Inventive Example   |
| 36  | 150                       | 150                       | 50                                          | 150                              | Inventive Example   |
| 37  | 150                       | 150                       | 50                                          | 150                              | Inventive Example   |

TABLE 4-continued

|    |     |     |     |     |                     |
|----|-----|-----|-----|-----|---------------------|
| 38 | 150 | 150 | 50  | 150 | Comparative Example |
| 39 | 150 | 150 | 50  | 150 | Inventive Example   |
| 40 | 150 | 150 | 50  | 150 | Comparative Example |
| 41 | 150 | 150 | 50  | 150 | Inventive Example   |
| 42 | 150 | 150 | 90  | 150 | Inventive Example   |
| 43 | 150 | 150 | 50  | 150 | Inventive Example   |
| 44 | 150 | 150 | 150 | 150 | Comparative Example |

\*1: The surface temperature of the steel sheet when it was restrained by the rolls.

\*2: The depression amount of each of the two rolls.

\*3: The inter-roll distance between the two rolls.

TABLE 5

| No. | Steel type | Sheet thickness mm | rolling<br>Rolling<br>reduction<br>% | Annealing<br>temperature<br>° C. | Annealing conditions                    |                                           |            |          |
|-----|------------|--------------------|--------------------------------------|----------------------------------|-----------------------------------------|-------------------------------------------|------------|----------|
|     |            |                    |                                      |                                  | Annealing<br>holding<br>time<br>Seconds | Quenching<br>start<br>temperature<br>° C. | *1<br>° C. | *2<br>mm |
| 45  | N          | 1.4                | 56                                   | 876                              | 60                                      | 757                                       | 300        | 0.5 30   |
| 46  |            | 1.4                | 56                                   | 895                              | 60                                      | 824                                       | —          | —        |
| 47  |            | 1.4                | 56                                   | 895                              | 60                                      | 824                                       | 300        | 0.5 30   |
| 48  |            | 1.4                | 56                                   | 884                              | 60                                      | 754                                       | 300        | 0.5 30   |
| 49  | O          | 1.4                | 56                                   | 881                              | 60                                      | 694                                       | 300        | 0.5 15   |
| 50  |            | 1.4                | 56                                   | 877                              | 60                                      | 877                                       | 300        | 0.5 15   |
| 51  |            | 1.4                | 56                                   | 877                              | 60                                      | 877                                       | 300        | 0.5 15   |
| 52  |            | 1.4                | 56                                   | 876                              | 60                                      | 793                                       | 300        | 0.5 15   |
| 53  | P          | 1.4                | 56                                   | 863                              | 20                                      | 753                                       | 300        | 0.5 15   |
| 54  |            | 1.4                | 56                                   | 877                              | 32                                      | 848                                       | 300        | 0.5 15   |
| 55  |            | 1.4                | 56                                   | 877                              | 240                                     | 848                                       | 300        | 0.5 15   |
| 56  |            | 1.4                | 56                                   | 871                              | 600                                     | 766                                       | 300        | 0.5 15   |
| 57  | Q          | 1.4                | 56                                   | 872                              | 60                                      | 845                                       | 300        | 0.5 2    |
| 58  |            | 1.4                | 56                                   | 871                              | 60                                      | 788                                       | 300        | 0.5 5    |
| 59  |            | 1.4                | 56                                   | 871                              | 60                                      | 788                                       | 300        | 0.5 15   |
| 60  |            | 1.4                | 56                                   | 892                              | 60                                      | 783                                       | 300        | 0.5 30   |
| 61  | R          | 1.4                | 56                                   | 890                              | 60                                      | 882                                       | 300        | 0.1 15   |
| 62  |            | 1.4                | 56                                   | 881                              | 60                                      | 875                                       | 300        | 0.4 15   |
| 63  |            | 1.4                | 56                                   | 881                              | 60                                      | 875                                       | 300        | 1.1 15   |
| 64  |            | 1.4                | 56                                   | 860                              | 60                                      | 684                                       | 300        | 1.5 15   |
| 65  | S          | 1.4                | 56                                   | 877                              | 60                                      | 705                                       | 300        | 0.5 20   |
| 66  |            | 1.4                | 56                                   | 898                              | 60                                      | 755                                       | 300        | 0.5 10   |
| 67  |            | 1.4                | 56                                   | 898                              | 60                                      | 755                                       | 300        | 0.5 30   |
| 68  |            | 1.4                | 56                                   | 894                              | 60                                      | 702                                       | 300        | 0.5 30   |
| 69  | T          | 1.4                | 56                                   | 898                              | 60                                      | 880                                       | 500        | 0.5 30   |
| 70  |            | 1.4                | 56                                   | 869                              | 60                                      | 743                                       | 350        | 0.5 30   |
| 71  |            | 1.4                | 56                                   | 869                              | 60                                      | 743                                       | 50         | 0.5 30   |
| 72  |            | 1.4                | 56                                   | 899                              | 60                                      | 686                                       | 560        | 0.5 30   |
| 73  | U          | 1.4                | 56                                   | 898                              | 60                                      | 896                                       | 300        | 0.5 30   |
| 74  | V          | 1.4                | 56                                   | 886                              | 60                                      | 700                                       | 300        | 0.5 30   |
| 75  | W          | 1.4                | 56                                   | 890                              | 60                                      | 838                                       | 300        | 0.5 30   |
| 76  | X          | 1.4                | 56                                   | 893                              | 60                                      | 740                                       | 300        | 0.5 30   |
| 77  | Y          | 1.4                | 56                                   | 895                              | 60                                      | 804                                       | 250        | 0.5 30   |
| 78  | Z          | 1.4                | 56                                   | 898                              | 60                                      | 831                                       | 300        | 0.5 30   |
| 79  | AA         | 1.4                | 56                                   | 890                              | 60                                      | 807                                       | 300        | 0.5 30   |
| 80  | AB         | 1.4                | 56                                   | 890                              | 60                                      | 807                                       | 300        | 0.5 30   |
| 81  | AC         | 1.4                | 56                                   | 873                              | 60                                      | 829                                       | 300        | 0.5 30   |
| 82  | AD         | 1.4                | 56                                   | 880                              | 60                                      | 760                                       | 210        | 0.3 10   |
| 83  | AE         | 1.4                | 56                                   | 880                              | 60                                      | 650                                       | 340        | 0.3 10   |
| 84  | AF         | 1.4                | 56                                   | 880                              | 60                                      | 730                                       | 260        | 1.2 10   |
| 85  | AG         | 1.4                | 56                                   | 880                              | 60                                      | 760                                       | 250        | 0.6 10   |
| 86  | AH         | 1.4                | 56                                   | 880                              | 60                                      | 730                                       | 200        | 0.6 10   |
| 87  | AI         | 1.4                | 56                                   | 880                              | 60                                      | 730                                       | 260        | 0.6 6    |
| 88  | AJ         | 1.4                | 56                                   | 880                              | 60                                      | 730                                       | 160        | 0.6 3    |
| 89  | AK         | 1.4                | 56                                   | 880                              | 60                                      | 730                                       | 230        | 0.6 3    |

| No. | Annealing conditions      |                           |                                             |                                  |                     |
|-----|---------------------------|---------------------------|---------------------------------------------|----------------------------------|---------------------|
|     | Roll diameter<br>Rn<br>mm | Roll diameter<br>rn<br>mm | Watercooling<br>stop<br>temperature<br>° C. | Reheating<br>temperature<br>° C. | Remarks             |
| 45  | 300                       | 300                       | 50                                          | 150                              | Inventive Example   |
| 46  | —                         | —                         | 50                                          | 200                              | Comparative Example |
| 47  | 300                       | 300                       | 50                                          | 250                              | Inventive Example   |
| 48  | 300                       | 300                       | 50                                          | 320                              | Comparative Example |

TABLE 5-continued

|    |      |     |    |     |                     |
|----|------|-----|----|-----|---------------------|
| 49 | 150  | 150 | 50 | 80  | Comparative Example |
| 50 | 150  | 150 | 50 | 180 | Inventive Example   |
| 51 | 150  | 150 | 50 | 320 | Comparative Example |
| 52 | 150  | 150 | 50 | 120 | Inventive Example   |
| 53 | 150  | 150 | 50 | 150 | Comparative Example |
| 54 | 150  | 150 | 50 | 150 | Inventive Example   |
| 55 | 150  | 150 | 50 | 150 | Inventive Example   |
| 56 | 150  | 150 | 50 | 150 | Inventive Example   |
| 57 | 150  | 150 | 50 | 150 | Inventive Example   |
| 58 | 150  | 150 | 50 | 150 | Inventive Example   |
| 59 | 150  | 150 | 50 | 150 | Inventive Example   |
| 60 | 150  | 150 | 50 | 150 | Comparative Example |
| 61 | 150  | 150 | 50 | 150 | Inventive Example   |
| 62 | 150  | 150 | 50 | 150 | Inventive Example   |
| 63 | 150  | 150 | 50 | 150 | Inventive Example   |
| 64 | 150  | 150 | 50 | 150 | Comparative Example |
| 65 | 60   | 300 | 50 | 150 | Inventive Example   |
| 66 | 200  | 40  | 50 | 150 | Comparative Example |
| 67 | 800  | 400 | 50 | 150 | Inventive Example   |
| 68 | 1200 | 500 | 50 | 150 | Comparative Example |
| 69 | 300  | 300 | 50 | 150 | Inventive Example   |
| 70 | 300  | 300 | 50 | 150 | Inventive Example   |
| 71 | 300  | 300 | 50 | 150 | Inventive Example   |
| 72 | 300  | 300 | 50 | 150 | Comparative Example |
| 73 | 300  | 300 | 50 | 150 | Comparative Example |
| 74 | 300  | 300 | 50 | 150 | Comparative Example |
| 75 | 300  | 300 | 50 | 150 | Comparative Example |
| 76 | 300  | 300 | 50 | 150 | Comparative Example |
| 77 | 300  | 300 | 50 | 150 | Comparative Example |
| 78 | 300  | 300 | 50 | 150 | Comparative Example |
| 79 | 300  | 300 | 50 | 150 | Comparative Example |
| 80 | 300  | 300 | 50 | 150 | Comparative Example |
| 81 | 300  | 300 | 50 | 150 | Comparative Example |
| 82 | 150  | 150 | 50 | 170 | Inventive Example   |
| 83 | 150  | 150 | 50 | 170 | Inventive Example   |
| 84 | 150  | 150 | 50 | 170 | Inventive Example   |
| 85 | 150  | 150 | 50 | 170 | Inventive Example   |
| 86 | 150  | 150 | 50 | 170 | Inventive Example   |
| 87 | 150  | 150 | 50 | 170 | Inventive Example   |
| 88 | 150  | 150 | 50 | 170 | Inventive Example   |
| 89 | 150  | 150 | 50 | 170 | Inventive Example   |

\*1: The surface temperature of the steel sheet when it was restrained by the rolls.

\*2: The depression amount of each of the two rolls.

\*3: The inter-roll distance between the two rolls.

## 2. Evaluation Methods

For each of the steel sheets obtained under various production conditions, the steel microstructure was analyzed to examine microstructure fractions, and a tensile test was performed to evaluate tensile properties such as tensile strength. Moreover, the warpage of the steel sheet was used

40 to evaluate the shape uniformity, and X-ray diffraction measurement was performed to examine the dislocation density in the metal phases. The evaluation methods are the same as those in Example 1.

## 3. Evaluation Results

The results of the evaluation are shown in Tables 6 and 7.

TABLE 6

| No. | Steel type | Microstructure |     |          | Transformation temperature<br>Ms<br>° C. | Tensile properties |      |        | Shape  |       | Remarks |
|-----|------------|----------------|-----|----------|------------------------------------------|--------------------|------|--------|--------|-------|---------|
|     |            | M %            | F % | Others % |                                          | *1 %               | *2 % | YS MPa | TS MPa | AYR % |         |
| 1   | A          | 30             | 66  | 4        | 392                                      | 124                | 127  | 648    | 772    | 0     | 5       |
| 2   |            | 35             | 62  | 3        | 402                                      | 128                | 122  | 657    | 782    | -1    | 3       |
| 3   |            | 32             | 67  | 1        | 396                                      | 95                 | 99   | 651    | 775    | 6     | 22      |
| 4   |            | 36             | 62  | 2        | 404                                      | 134                | 120  | 640    | 780    | -1    | 4       |
| 5   | B          | 42             | 56  | 2        | 450                                      | 124                | 128  | 824    | 981    | 0     | 5       |
| 6   |            | 48             | 49  | 3        | 462                                      | 123                | 123  | 822    | 990    | 1     | 7       |
| 7   |            | 45             | 50  | 5        | 456                                      | 126                | 123  | 838    | 986    | 1     | 4       |
| 8   |            | 40             | 56  | 4        | 446                                      | 108                | 117  | 813    | 980    | 2     | 3       |
| 9   | C          | 55             | 42  | 3        | 365                                      | 116                | 126  | 1000   | 1220   | -1    | 16      |
| 10  |            | 59             | 39  | 2        | 371                                      | 103                | 131  | 1028   | 1224   | -1    | 4       |
| 11  |            | 56             | 42  | 2        | 367                                      | 120                | 131  | 976    | 1220   | -1    | 5       |
| 12  |            | 53             | 42  | 5        | 362                                      | 129                | 126  | 1020   | 1214   | -1    | 3       |
| 13  | D          | 84             | 14  | 2        | 398                                      | 129                | 126  | 1165   | 1438   | 1     | 5       |
| 14  |            | 86             | 9   | 5        | 400                                      | 129                | 126  | 1182   | 1442   | 0     | 5       |
| 15  |            | 90             | 7   | 3        | 404                                      | 125                | 129  | 1233   | 1451   | -1    | 2       |
| 16  |            | 85             | 12  | 3        | 399                                      | 98                 | 110  | 1167   | 1441   | 4     | 5       |

40 to evaluate the shape uniformity, and X-ray diffraction measurement was performed to examine the dislocation density in the metal phases. The evaluation methods are the same as those in Example 1.

## 3. Evaluation Results

The results of the evaluation are shown in Tables 6 and 7.

TABLE 6-continued

| No. | Steel type | Microstructure |     |          | Transformation temperature |      | Tensile properties |        |        | Shape Maximum |            |                     |
|-----|------------|----------------|-----|----------|----------------------------|------|--------------------|--------|--------|---------------|------------|---------------------|
|     |            | M %            | F % | Others % | Ms °C.                     | *1 % | *2 %               | YS MPa | TS MPa | ΔYR %         | warpage mm | Remarks             |
| 17  | E          | 98             | 2   | 0        | 417                        | 120  | 129                | 1277   | 1538   | -1            | 2          | Inventive Example   |
| 18  |            | 93             | 5   | 2        | 412                        | 125  | 120                | 1300   | 1529   | -1            | 11         | Inventive Example   |
| 19  |            | 92             | 6   | 2        | 411                        | 119  | 115                | 1068   | 1257   | 2             | 5          | Inventive Example   |
| 20  |            | 99             | 1   | 0        | 418                        | 99   | 119                | 1030   | 1241   | 4             | 3          | Comparative Example |
| 21  | F          | 93             | 2   | 5        | 385                        | 128  | 128                | 1404   | 1733   | -1            | 18         | Comparative Example |
| 22  |            | 97             | 3   | 0        | 389                        | 126  | 125                | 1465   | 1744   | 1             | 4          | Inventive Example   |
| 23  |            | 93             | 5   | 2        | 385                        | 122  | 124                | 1440   | 1735   | -1            | 5          | Inventive Example   |
| 24  |            | 100            | 0   | 0        | 392                        | 125  | 122                | 1398   | 1748   | 1             | 3          | Inventive Example   |
| 25  | G          | 96             | 3   | 1        | 358                        | 123  | 122                | 1395   | 1701   | -1            | 17         | Comparative Example |
| 26  |            | 95             | 1   | 4        | 357                        | 122  | 126                | 1409   | 1697   | -2            | 7          | Inventive Example   |
| 27  |            | 100            | 0   | 0        | 361                        | 125  | 122                | 1436   | 1709   | 0             | 5          | Inventive Example   |
| 28  |            | 94             | 3   | 3        | 356                        | 128  | 130                | 1424   | 1695   | -1            | 3          | Inventive Example   |
| 29  | H          | 98             | 2   | 0        | 368                        | 127  | 128                | 1899   | 2288   | 1             | 12         | Inventive Example   |
| 30  |            | 96             | 0   | 4        | 365                        | 122  | 127                | 1843   | 2275   | 0             | 10         | Inventive Example   |
| 31  |            | 95             | 1   | 4        | 363                        | 120  | 123                | 1909   | 2273   | 1             | 11         | Inventive Example   |
| 32  | I          | 48             | 48  | 4        | 146                        | 123  | 137                | 1211   | 1495   | -3            | 9          | Inventive Example   |
| 33  | J          | 98             | 2   | 0        | 394                        | 126  | 138                | 1414   | 1724   | -2            | 5          | Inventive Example   |
| 34  |            | 97             | 0   | 3        | 393                        | 128  | 147                | 1412   | 1722   | -5            | 5          | Comparative Example |
| 35  |            | 96             | 4   | 0        | 392                        | 124  | 137                | 1445   | 1720   | -3            | 2          | Inventive Example   |
| 36  | K          | 99             | 1   | 0        | 391                        | 128  | 138                | 1371   | 1714   | -2            | 5          | Inventive Example   |
| 37  |            | 96             | 4   | 0        | 388                        | 124  | 137                | 1418   | 1708   | -2            | 8          | Inventive Example   |
| 38  |            | 96             | 4   | 0        | 388                        | 125  | 136                | 1450   | 1706   | -1            | 17         | Comparative Example |
| 39  | L          | 94             | 6   | 0        | 378                        | 124  | 129                | 1127   | 1374   | 0             | 7          | Inventive Example   |
| 40  |            | 93             | 6   | 1        | 378                        | 124  | 129                | 1123   | 1370   | -1            | 17         | Comparative Example |
| 41  |            | 93             | 3   | 4        | 378                        | 130  | 130                | 1122   | 1368   | -1            | 13         | Inventive Example   |
| 42  | M          | 85             | 13  | 2        | 368                        | 127  | 137                | 1154   | 1358   | -1            | 11         | Inventive Example   |
| 43  |            | 90             | 8   | 2        | 372                        | 137  | 139                | 1132   | 1364   | -1            | 5          | Inventive Example   |
| 44  |            | 91             | 4   | 5        | 372                        | 128  | 137                | 1160   | 1365   | -2            | 17         | Comparative Example |

M: Area fraction of martensite,

F: Area fraction of ferrite,

Others: Area fraction of other metal phases

\*1: The ratio of the dislocation density in the metal phases at the widthwise edge of the sheet to the dislocation density in the metal phases at the widthwise center of the sheet on the surface of the steel sheet (the dislocation density on the surface of the widthwise edge of the sheet/the dislocation density on the surface of the widthwise center of the sheet).

\*2: The ratio of the dislocation density in the metal phases at the widthwise edge of the sheet to the dislocation density in the metal phases at the widthwise center of the sheet at the thicknesswise center of the sheet (the dislocation density in the thicknesswise central portion at the widthwise edge of the sheet/the dislocation density in the thicknesswise central portion at the widthwise center of the sheet).

TABLE 7

| No. | Steel type | Microstructure |     |          | Transformation temperature |      | Tensile properties |        |        | Shape Maximum |            |                     |
|-----|------------|----------------|-----|----------|----------------------------|------|--------------------|--------|--------|---------------|------------|---------------------|
|     |            | M %            | F % | Others % | Ms °C.                     | *1 % | *2 %               | YS MPa | TS MPa | ΔYR %         | warpage mm | Remarks             |
| 45  | N          | 90             | 6   | 4        | 388                        | 123  | 129                | 1357   | 1635   | 0             | 5          | Inventive Example   |
| 46  |            | 94             | 2   | 4        | 392                        | 94   | 95                 | 1363   | 1642   | 6             | 25         | Comparative Example |
| 47  |            | 98             | 1   | 1        | 396                        | 122  | 125                | 1384   | 1648   | -1            | 12         | Inventive Example   |
| 48  |            | 95             | 1   | 4        | 393                        | 120  | 130                | 1397   | 1643   | 1             | 19         | Comparative Example |
| 49  | O          | 98             | 2   | 0        | 395                        | 142  | 143                | 1296   | 1581   | -5            | 5          | Comparative Example |
| 50  |            | 96             | 0   | 4        | 394                        | 128  | 131                | 1275   | 1574   | -1            | 3          | Inventive Example   |
| 51  |            | 96             | 2   | 2        | 394                        | 129  | 137                | 1339   | 1575   | -2            | 18         | Comparative Example |
| 52  |            | 95             | 0   | 5        | 393                        | 136  | 137                | 1258   | 1573   | -2            | 1          | Inventive Example   |
| 53  | P          | 96             | 2   | 2        | 410                        | 120  | 141                | 1362   | 1622   | -4            | 5          | Comparative Example |
| 54  |            | 96             | 1   | 3        | 410                        | 123  | 137                | 1315   | 1623   | -3            | 5          | Inventive Example   |
| 55  |            | 97             | 1   | 2        | 411                        | 126  | 130                | 1381   | 1625   | -1            | 2          | Inventive Example   |
| 56  |            | 97             | 2   | 1        | 411                        | 128  | 133                | 1299   | 1624   | -2            | 5          | Inventive Example   |
| 57  | Q          | 94             | 5   | 1        | 407                        | 120  | 125                | 1353   | 1670   | -1            | 5          | Inventive Example   |
| 58  |            | 96             | 1   | 3        | 409                        | 124  | 128                | 1390   | 1675   | -2            | 3          | Inventive Example   |
| 59  |            | 98             | 1   | 1        | 412                        | 128  | 135                | 1425   | 1677   | -1            | 5          | Inventive Example   |
| 60  |            | 98             | 2   | 0        | 412                        | 94   | 118                | 1357   | 1675   | 5             | 5          | Comparative Example |
| 61  | R          | 90             | 10  | 0        | 396                        | 129  | 123                | 1082   | 1273   | 0             | 4          | Inventive Example   |
| 62  |            | 87             | 13  | 0        | 394                        | 122  | 123                | 1064   | 1267   | 1             | 5          | Inventive Example   |
| 63  |            | 88             | 7   | 5        | 394                        | 118  | 114                | 1078   | 1268   | 2             | 4          | Inventive Example   |
| 64  |            | 87             | 8   | 5        | 394                        | 95   | 108                | 1065   | 1268   | 5             | 3          | Comparative Example |
| 65  | S          | 98             | 2   | 0        | 394                        | 124  | 126                | 1172   | 1412   | -1            | 5          | Inventive Example   |
| 66  |            | 90             | 9   | 1        | 388                        | 130  | 125                | 1121   | 1401   | -1            | 17         | Comparative Example |
| 67  |            | 91             | 7   | 2        | 389                        | 123  | 124                | 1193   | 1403   | 1             | 5          | Inventive Example   |
| 68  |            | 92             | 6   | 2        | 390                        | 126  | 124                | 1137   | 1404   | 1             | 18         | Comparative Example |
| 69  | T          | 97             | 1   | 2        | 379                        | 121  | 120                | 1364   | 1663   | 1             | 14         | Inventive Example   |

TABLE 7-continued

| No. | Steel type | Microstructure |     |          | Transformation temperature<br>° C. | Tensile properties |      |        | Shape Maximum |       |            |                     |
|-----|------------|----------------|-----|----------|------------------------------------|--------------------|------|--------|---------------|-------|------------|---------------------|
|     |            | M %            | F % | Others % |                                    | *1 %               | *2 % | YS MPa | TS MPa        | AYR % | warpage mm | Remarks             |
| 70  |            | 96             | 4   | 0        | 379                                | 129                | 128  | 1395   | 1661          | 1     | 5          | Inventive Example   |
| 71  |            | 94             | 1   | 5        | 377                                | 127                | 124  | 1393   | 1658          | -1    | 5          | Inventive Example   |
| 72  |            | 97             | 2   | 1        | 379                                | 127                | 123  | 1330   | 1662          | 0     | 18         | Comparative Example |
| 73  | U          | 99             | 0   | 1        | 279                                | 120                | 124  | 2789   | 3320          | 1     | 20         | Comparative Example |
| 74  | V          | 14             | 86  | 0        | 402                                | 120                | 121  | 404    | 475           | 0     | 4          | Comparative Example |
| 75  | W          | 89             | 9   | 2        | 425                                | 130                | 141  | 1037   | 1280          | -4    | 5          | Comparative Example |
| 76  | X          | 95             | 4   | 1        | 333                                | 122                | 141  | 1452   | 1815          | -5    | 3          | Comparative Example |
| 77  | Y          | 18             | 82  | 0        | 120                                | 124                | 124  | 604    | 710           | -1    | 5          | Comparative Example |
| 78  | Z          | 91             | 5   | 4        | 394                                | 123                | 147  | 1381   | 1684          | -4    | 4          | Comparative Example |
| 79  | AA         | 94             | 2   | 4        | 400                                | 126                | 149  | 1315   | 1604          | -5    | 5          | Comparative Example |
| 80  | AB         | 96             | 2   | 2        | 406                                | 130                | 148  | 1288   | 1552          | -4    | 5          | Comparative Example |
| 81  | AC         | 93             | 4   | 3        | 420                                | 129                | 150  | 1090   | 1346          | -5    | 5          | Comparative Example |
| 82  | AD         | 98             | 0   | 2        | 423                                | 122                | 118  | 1226   | 1482          | 1     | 3          | Inventive Example   |
| 83  | AE         | 98             | 0   | 2        | 412                                | 124                | 126  | 1243   | 1488          | 0     | 2          | Inventive Example   |
| 84  | AF         | 98             | 0   | 2        | 416                                | 122                | 124  | 1230   | 1476          | 2     | 2          | Inventive Example   |
| 85  | AG         | 98             | 0   | 2        | 429                                | 126                | 131  | 1246   | 1491          | -2    | 3          | Inventive Example   |
| 86  | AH         | 98             | 0   | 2        | 423                                | 125                | 120  | 1239   | 1483          | 0     | 4          | Inventive Example   |
| 87  | AI         | 98             | 0   | 2        | 409                                | 125                | 126  | 1242   | 1496          | 0     | 4          | Inventive Example   |
| 88  | AJ         | 98             | 0   | 2        | 423                                | 124                | 122  | 1250   | 1510          | 1     | 2          | Inventive Example   |
| 89  | AK         | 98             | 0   | 2        | 418                                | 120                | 130  | 1252   | 1516          | 0     | 3          | Inventive Example   |

M: Area fraction of martensite,

F: Area fraction of ferrite,

Others: Area fraction of other metal phases

\*1: The ratio of the dislocation density in the metal phases at the widthwise edge of the sheet to the dislocation density in the metal phases at the widthwise center of the sheet on the surface of the steel sheet (the dislocation density on the surface of the widthwise edge of the sheet/the dislocation density on the surface of the widthwise center of the sheet).

\*2: The ratio of the dislocation density in the metal phases at the widthwise center of the sheet at the thicknesswise center of the sheet to the dislocation density in the metal phases at the widthwise center of the sheet at the thicknesswise central portion at the widthwise edge of the sheet/the dislocation density in the thicknesswise central portion at the widthwise center of the sheet).

In the present Example, a steel sheet was rated pass when the TS was 750 MPa or more, the AYR was from -3% to 3%, and the maximum amount of warpage was 15 mm or less and shown as Inventive Example in Table 6 or 7. 35 However, a steel sheet was rated fail when at least one of the above conditions was not satisfied and shown as Comparative Example in Table 6 or 7.

### Example 3

The steel sheet No. 1 in Table 6 in Example 2 was subjected to press-forming to produce a member in an Inventive Example. Moreover, the steel sheet No. 1 in Table 6 in Example 2 and the steel sheet No. 2 in Table 6 in Example 2 were joined together by spot welding to produce a member in another Inventive Example. These members in the Inventive Examples had high strength, and their dimensional accuracy was high. It was therefore found that these members can be preferably used for automotive parts etc. 50

### REFERENCE SIGNS LIST

10 steel sheet

11a roll

11b roll

12 cooling water

A1 inter-roll distance between two rolls

D1 conveying direction of steel sheet

The invention claimed is:

1. A steel sheet comprising a steel microstructure containing: in area fraction, martensite: from 20% to 100%, ferrite: from 0% to 80%, and another metal phase: 5% or less; 65 in which, on a surface of the steel sheet, a ratio of a dislocation density in metal phases at a widthwise edge

of the steel sheet to a dislocation density in the metal phases at a widthwise center of the steel sheet is from 100% to 140%; and

in which, at a thicknesswise center of the steel sheet, a ratio of a dislocation density in the metal phases at the widthwise edge of the steel sheet to a dislocation density in the metal phases at the widthwise center of the steel sheet is from 100% to 140%,

wherein the maximum amount of warpage of the steel sheet when the steel sheet is sheared to a length of 1 m in a rolling direction is 15 mm or less.

2. The steel sheet according to claim 1, having a chemical composition containing, in mass %,

C: from 0.05% to 0.60%,

Si: from 0.01% to 2.0%,

Mn: from 0.1% to 3.2%,

P: 0.050% or less,

S: 0.0050% or less,

Al: from 0.005% to 0.10%, and

N: 0.010% or less, with the balance being Fe and incidental impurities.

3. The steel sheet according to claim 2, wherein the chemical composition further contains at least one selected from following groups A to E consisting of:

Group A: in mass %, at least one selected from

Cr: 0.20% or less,

Mo: less than 0.15%, and

V: 0.05% or less;

Group B: in mass %, at least one selected from

Nb: 0.020% or less and

Ti: 0.020% or less;

Group C: in mass %, at least one selected from

Cu: 0.20% or less and

Ni: 0.10% or less;

Group D: in mass %,

B: less than 0.0020%;

Group E: in mass %, at least one selected from

Sb: 0.1% or less and

Sn: 0.1% or less.

4. A member prepared by subjecting the steel sheet according to claim 1 to at least one of forming and welding.

5. A member prepared by subjecting the steel sheet according to claim 2 to at least one of forming and welding.

6. A member prepared by subjecting the steel sheet according to claim 3 to at least one of forming and welding.

7. A method for producing a steel sheet, the method comprising:

a hot rolling step of heating a steel slab having the chemical composition according to claim 2 and then 15 hot-rolling the steel slab; and

an annealing step of holding a hot-rolled steel sheet obtained in the hot rolling step at an annealing temperature equal to or higher than  $A_{C1}$  temperature for 30 seconds or longer, then starting water quenching the 20 hot-rolled steel sheet from a temperature equal to or higher than Ms temperature including water cooling to 100° C. or lower, and reheating the hot-rolled steel sheet to from 100° C. to 300° C.,

wherein, in a region in which a surface temperature of the 25 steel sheet is equal to or lower than (Ms temperature+150° C.) during the water cooling in the water quenching in the annealing step, the steel sheet is restrained from front and back sides of the steel sheet using two rolls such that the following conditions (1) to (3) are satisfied, the two rolls being disposed with the steel sheet interposed therebetween:

(1) a depression amount of each of the two rolls is more 30 than 0 mm and t mm or less, where t is a thickness of the steel sheet;

(2)  $R_n$  and  $r_n$  are from 50 mm to 1000 mm, where  $R_n$  and 35  $r_n$  are roll diameters of the respective two rolls; and

(3) an inter-roll distance between the two rolls is more than 0 mm and  $(R_n+r_n+t)/16$  mm or less.

8. A method for producing a steel sheet, the method 40 comprising:

a hot rolling step of heating a steel slab having the chemical composition according to claim 3 and then hot-rolling the steel slab; and

an annealing step of holding a hot-rolled steel sheet 45 obtained in the hot rolling step at an annealing temperature equal to or higher than  $A_{C1}$  temperature for 30 seconds or longer, then starting water quenching the hot-rolled steel sheet from a temperature equal to or higher than Ms temperature including water cooling to 100° C. or lower, and reheating the hot-rolled steel sheet to from 100° C. to 300° C.,

wherein, in a region in which a surface temperature of the 50 steel sheet is equal to or lower than (Ms temperature+150° C.) during the water cooling in the water quenching in the annealing step, the steel sheet is restrained from front and back sides of the steel sheet using two rolls such that the following conditions (1) to (3) are satisfied, the two rolls being disposed with the steel sheet interposed therebetween:

(1) a depression amount of each of the two rolls is more 55 than 0 mm and t mm or less, where t is a thickness of the steel sheet;

(2)  $R_n$  and  $r_n$  are from 50 mm to 1000 mm, where  $R_n$  and 60  $r_n$  are roll diameters of the respective two rolls; and

(3) an inter-roll distance between the two rolls is more than 0 mm and  $(R_n+r_n+t)/16$  mm or less.

9. A method for producing a steel sheet, the method comprising:

a hot rolling step of heating a steel slab having the chemical composition according to claim 2 and then hot-rolling the steel slab;

a cold rolling step of cold-rolling a hot-rolled steel sheet obtained in the hot rolling step; and

an annealing step of holding a cold-rolled steel sheet obtained in the cold rolling step at an annealing temperature equal to or higher than  $A_{C1}$  temperature for 30 seconds or longer, then starting water quenching the cold-rolled steel sheet from a temperature equal to or higher than Ms temperature including water cooling to 100° C. or lower, and reheating the cold-rolled steel sheet to from 100° C. to 300° C.,

wherein, in a region in which a surface temperature of the steel sheet is equal to or lower than (Ms temperature+150° C.) during the water cooling in the water quenching in the annealing step, the steel sheet is restrained from front and back sides of the steel sheet using two rolls such that the following conditions (1) to (3) are satisfied, the two rolls being disposed with the steel sheet interposed therebetween:

(1) a depression amount of each of the two rolls is more than 0 mm and t mm or less, where t is a thickness of the steel sheet;

(2)  $R_n$  and  $r_n$  are from 50 mm to 1000 mm, where  $R_n$  and 45  $r_n$  are roll diameters of the respective two rolls; and

(3) an inter-roll distance between the two rolls is more than 0 mm and  $(R_n+r_n+t)/16$  mm or less.

10. A method for producing a steel sheet, the method comprising:

a hot rolling step of heating a steel slab having the chemical composition according to claim 3 and then hot-rolling the steel slab;

a cold rolling step of cold-rolling a hot-rolled steel sheet obtained in the hot rolling step; and

an annealing step of holding a cold-rolled steel sheet obtained in the cold rolling step at an annealing temperature equal to or higher than  $A_{C1}$  temperature for 30 seconds or longer, then starting water quenching the cold-rolled steel sheet from a temperature equal to or higher than Ms temperature including water cooling to 100° C. or lower, and reheating the cold-rolled steel sheet to from 100° C. to 300° C.,

wherein, in a region in which a surface temperature of the steel sheet is equal to or lower than (Ms temperature+150° C.) during the water cooling in the water quenching in the annealing step, the steel sheet is restrained from front and back sides of the steel sheet using two rolls such that the following conditions (1) to (3) are satisfied, the two rolls being disposed with the steel sheet interposed therebetween:

(1) a depression amount of each of the two rolls is more than 0 mm and t mm or less, where t is a thickness of the steel sheet;

(2)  $R_n$  and  $r_n$  are from 50 mm to 1000 mm, where  $R_n$  and 65  $r_n$  are roll diameters of the respective two rolls; and

(3) an inter-roll distance between the two rolls is more than 0 mm and  $(R_n+r_n+t)/16$  mm or less.

11. A method for producing a member, the method comprising the step of subjecting the steel sheet produced by the steel sheet production method according to claim 7 to at least one of forming and welding.

12. A method for producing a member, the method comprising the step of subjecting the steel sheet produced by

the steel sheet production method according to claim **8** to at least one of forming and welding.

**13.** A method for producing a member, the method comprising the step of subjecting the steel sheet produced by the steel sheet production method according to claim **9** to at least one of forming and welding. 5

**14.** A method for producing a member, the method comprising the step of subjecting the steel sheet produced by the steel sheet production method according to claim **10** to at least one of forming and welding. 10

\* \* \* \* \*